# EUROPEAN PATENT SPECIFICATION

(11) **EP 2 656 882 B1**
(45) Date of publication and mention of the grant of the patent: **09.06.2021**
(21) Application number: 13164343.9
(22) Date of filing: 18.04.2013
(51) Int. Cl.: A63B 37/00

(54) **Golf ball**
Golfball
Balle de golf

(30) Priority: 25.04.2012 JP 2012099641; 22.05.2012 JP 2012116542; 24.05.2012 JP 2012118422; 24.05.2012 JP 2012118544; 31.05.2012 JP 2012124249; 31.05.2012 JP 2012124924
(43) Date of publication of application: 30.10.2013
(62) Divisional of application: 17192516.7
(73) Proprietor: Sumitomo Rubber Industries, Ltd., Kobe-shi, Hyogo-ken (JP)
(72) Inventor: Isogawa, Kazuhiko, Kobe-shi, Hyogo 651-0072 (JP); Tachibana, Kosuke, Kobe-shi, Hyogo 651-0072 (JP)
(74) Representative: Manitz Finsterwald Patent- und Rechtsanwaltspartnerschaft mbB

(56) References cited:
- US-A1- 2008 146 377
- US-A1- 2009 227 394
- US-A1- 2010 273 575
- US-A1- 2011 159 998
- US-A1- 2012 088 604
- US-B2- 7 850 548

## Description

This application claims priority on Patent Application No. 2012-99641 filed in JAPAN on April 25, 2012, Patent Application No. 2012-116542 filed in JAPAN on May 22, 2012, Patent Application No. 2012-118422 filed in JAPAN on May 24, 2012, Patent Application No. 2012-118544 filed in JAPAN on May 24, 2012, Patent Application No. 2012-124924 filed in JAPAN on May 31, 2012, and Patent Application No. 2012-124249 filed in JAPAN on May 31, 2012.

### BACKGROUND OF THE INVENTION

### Field of the Invention

The present invention relates to golf balls. Specifically, the present invention relates to golf balls that include a solid core, a mid layer, and a cover.

### Description of the Related Art

Golf players' foremost requirement for golf balls is flight performance. In particular, golf players place importance on flight performance upon a shot with a driver. Flight performance correlates with the resilience performance of a golf ball. When a golf ball having excellent resilience performance is hit, the golf ball flies at a high speed, thereby achieving a large flight distance. Golf balls that include a core having excellent resilience performance are disclosed in JP61-37178, JP2008-212681 (US2008/0214324), JP2008-523952 (US2006/0135287 and US2007/0173607), and JP2009-119256 (US2009/0124757) .

The core disclosed in JP61-37178 is obtained from a rubber composition that includes a co-crosslinking agent and a crosslinking activator. This publication discloses palmitic acid, stearic acid, and myristic acid as the crosslinking activator.

The core disclosed in JP2008-212681 is obtained from a rubber composition that includes an organic peroxide, a metal salt of an α,β-unsaturated carboxylic acid, and a copper salt of a fatty acid.

The core disclosed in JP2008-523952 is obtained from a rubber composition that includes a metal salt of an unsaturated monocarboxylic acid, a free radical initiator, and a non-conjugated diene monomer.

The core disclosed in JP2009-119256 is obtained from a rubber composition that includes a polybutadiene whose vinyl content is equal to or less than 2%, whose cis 1,4-bond content is equal to or greater than 80%, and which has an active end modified with an alkoxysilane compound.

An appropriate trajectory height is required in order to achieve a large flight distance. A trajectory height depends on a spin rate and a launch angle. With a golf ball that achieves a high trajectory by a high spin rate, a flight distance is insufficient. With a golf ball that achieves a high trajectory by a high launch angle, a large flight distance is obtained. Use of an outer-hard/inner-soft structure in a golf ball can achieve a low spin rate and a high launch angle. Modifications regarding a hardness distribution of a core are disclosed in JP6-154357 (USP5,403,010), JP2008-194471 (USP7,344,455, US2008/0194358, US2008/0194359, and US2008/0214325), and JP2008-194473 (US2008/0194357 and US2008/0312008).

In the core disclosed in JP6-154357, a JIS-C hardness H1 at the central point of the core is 58 to 73, a JIS-C hardness H2 in a region that extends over a distance range from equal to or greater than 5 mm to equal to or less than 10 mm from the central point is equal to or greater than 65 but equal to or less than 75, a JIS-C hardness H3 at a point located at a distance of 15 mm from the central point is equal to or greater than 74 but equal to or less than 82, and a JIS-C hardness H4 at the surface of the core is equal to or greater than 76 but equal to or less than 84. The hardness H2 is greater than the hardness H1, the hardness H3 is greater than the hardness H2, and the hardness H4 is equal to or greater than the hardness H3.

In the core disclosed in JP2008-194471, a Shore D hardness at the central point of the core is equal to or greater than 30 but equal to or less than 48, a Shore D hardness at a point located at a distance of 4 mm from the central point is equal to or greater than 34 but equal to or less than 52, a Shore D hardness at a point located at a distance of 8 mm from the central point is equal to or greater than 40 but equal to or less than 58, a Shore D hardness at a point located at a distance of 12 mm from the central point is equal to or greater than 43 but equal to or less than 61, a Shore D hardness in a region that extends over a distance range from equal to or greater than 2 mm to equal to or less than 3 mm from the surface of the core is equal to or greater than 36 but equal to or less than 54, and a Shore D hardness at the surface is equal to or greater than 41 but equal to or less than 59.

In the core disclosed in JP2008-194473, a Shore D hardness at the central point of the core is equal to or greater than 25 but equal to or less than 45, a Shore D hardness in a region that extends over a distance range from equal to or greater than 5 mm to equal to or less than 10 mm from the central point is equal to or greater than 39 but equal to or less than 58, a Shore D hardness at a point located at a distance of 15 mm from the central point is equal to or greater than 36 but equal to or less than 55, and a Shore D hardness at the surface of the core is equal to or greater than 55 but equal to or less than 75.

JP2010-253268 (US2010/0273575) discloses a golf ball that includes a core, an envelope layer, a mid layer, and a cover. In the core, the hardness gradually increases from the central point of the core to the surface of the core. The difference between a JIS-C hardness at the surface and a JIS-C hardness at the central point is equal to or greater than 15. The hardness of the cover is greater than the hardness of the mid layer, and the hardness of the mid layer is greater than the hardness of the envelope layer.

US 2011/0159998 A1 discloses a golf ball having a four-layered structure, wherein e.g. the JIS-C hardness of the central point of the core is 60, the JIS-C hardness of the surface of the core is 85, the JIS-C hardness of the mid layer is 94 and the JIS-C hardness of the outer cover is between 45 and 56, respectively.

Golf players also place importance on controllability of golf balls. Controllability depends on spin rate. When a backspin rate is high, the run is short. It is easy for golf players to cause a golf ball, to which backspin is easily provided, to stop at a target point. When a sidespin rate is high, the golf ball tends to curve. It is easy for golf players to intentionally cause a golf ball, to which sidespin is easily provided, to curve. A golf ball to which spin is easily provided has excellent controllability. In particular, advanced golf players place importance on controllability upon a shot with a short iron.

Golf players are also interested in durability of golf balls. When being hit with a driver or the like, a golf ball receives great shock and deforms. When a local load is applied to a part of the ball due to the deformation, the golf ball is broken. A golf ball that is resistant to deformation caused by hitting can be continuously used over a long period of time.

As described above, when a golf ball having a high launch angle and a low spin rate is hit with a driver, a large flight distance is obtained. However, a golf ball having a low spin rate has inferior controllability. Golf players desire achievement of both a desired flight distance and desired controllability. Furthermore, a golf ball that has excellent durability against hitting and can be continuously used is desired. An object of the present invention is to provide a golf ball that has excellent flight performance upon a shot with a driver and excellent controllability upon a shot with a short iron and excellent durability.

### SUMMARY OF THE INVENTION

A golf ball according to the present invention includes a spherical core, an inner mid layer positioned outside the core, an outer mid layer positioned outside the inner mid layer, and a cover positioned outside the outer mid layer, wherein the core has a diameter of equal to or greater than 36.0 mm. When distances (%) from a central point of the core to nine points and JIS-C hardnesses at the nine points, which nine points are obtained by dividing a region from the central point of the core to a surface of the core at intervals of 12.5% of a radius of the core, are plotted in a graph, R² of a linear approximation curve obtained by a least-square method is equal to or greater than 0.95. A Shore D hardness Hm1 of the inner mid layer is greater than a Shore D hardness Hm2 of the outer mid layer. A Shore D hardness Hc of the cover is less than the hardness Hm1. A thickness T2 of the outer mid layer is equal to or greater than 0.5 mm but equal to or less than 1.6 mm. In the golf ball according to the present invention, a hardness distribution is appropriate. In the golf ball, the energy loss is low when being hit. The golf ball has excellent resilience performance. When the golf ball is hit with a driver, the spin rate is low. The great resilience performance and the low spin rate achieve a large flight distance. When the golf ball is hit with a short iron, the spin rate is high. The golf ball has excellent controllability. In the golf ball, the local load applied when being hit is low. The golf ball has excellent durability. Furthermore, in the golf ball, soft feel at impact is obtained.

According to another aspect, a golf ball according to the present invention includes a spherical core, an inner mid layer positioned outside the core, an outer mid layer positioned outside the inner mid layer, and a cover positioned outside the outer mid layer, wherein the core has a diameter of equal to or greater than 36.0 mm. When distances (%) from a central point of the core to nine points and JIS-Chardnesses at the nine points, which nine points are obtained by dividing a region from the central point of the core to a surface of the core at intervals of 12.5% of a radius of the core, are plotted in a graph, R² of a linear approximation curve obtained by a least-square method is equal to or greater than 0.95. A Shore D hardness Hm2 of the outer mid layer is greater than a Shore D hardness Hm1 of the inner mid layer. A Shore D hardness Hc of the cover is less than the hardness Hm2. The hardness Hm1 is less than 50. In the golf ball according to the present invention, a hardness distribution is appropriate. In the golf ball, the energy loss is low when being hit. The golf ball has excellent resilience performance. When the golf ball is hit with a driver, the spin rate is low. The great resilience performance and the low spin rate achieve a large flight distance. When the golf ball is hit with a short iron, the spin rate is high. The golf ball has excellent controllability. In the golf ball, the local load applied when being hit is low. The golf ball has excellent durability.

### BRIEF DESCRIPTION OF THE DRAWINGS

FIG. 1 is a partially cutaway cross-sectional view of a golf ball according to a first embodiment of the present invention;
FIG. 2 is a line graph showing a hardness distribution of a core of the golf ball in FIG. 1;
FIG. 3 is a partially cutaway cross-sectional view of a golf ball according to a second embodiment of the present invention;
FIG. 4 is a line graph showing a hardness distribution of a core of the golf ball in FIG. 3;

### DESCRIPTION OF THE PREFERRED EMBODIMENTS

The following will describe in detail the present invention, based on preferred embodiments with reference to the accompanying drawings.

### [First Embodiment]

A golf ball 2 shown in FIG. 1 includes a spherical core 4, an inner mid layer 6 positioned outside the core 4, an outer mid layer 8 positioned outside the inner mid layer 6, a reinforcing layer 10 positioned outside the outer mid layer 8, and a cover 12 positioned outside the reinforcing layer 10. On the surface of the cover 12, a large number of dimples 14 are formed. Of the surface of the golf ball 2, a part other than the dimples 14 is a land 16. The golf ball 2 includes a paint layer and a mark layer on the external side of the cover 12, but these layers are not shown in the drawing.

The golf ball 2 has a diameter of 40 mm or greater but 45 mm or less. From the standpoint of conformity to the rules established by the United States Golf Association (USGA), the diameter is preferably equal to or greater than 42.67 mm. In light of suppression of air resistance, the diameter is preferably equal to or less than 44 mm and more preferably equal to or less than 42.80 mm. The golf ball 2 has a weight of 40 g or greater but 50 g or less. In light of attainment of great inertia, the weight is preferably equal to or greater than 44 g and more preferably equal to or greater than 45.00 g. From the standpoint of conformity to the rules established by the USGA, the weight is preferably equal to or less than 45.93 g.

The core 4 is obtained by crosslinking a rubber composition. The rubber composition includes:
(a) a base rubber;
(b) a co-crosslinking agent;
(c) a crosslinking initiator; and
(d) an acid and/or a salt.

Examples of the base rubber (a) include polybutadienes, polyisoprenes, styrene-butadiene copolymers, ethylene-propylene-diene copolymers, and natural rubbers. In light of resilience performance, polybutadienes are preferred. When a polybutadiene and another rubber are used in combination, it is preferred that the polybutadiene is included as a principal component. Specifically, the proportion of the polybutadiene to the entire base rubber is preferably equal to or greater than 50% by weight and more preferably equal to or greater than 80% by weight. The proportion of cis-1, 4 bonds in the polybutadiene is preferably equal to or greater than 40% by weight and more preferably equal to or greater than 80% by weight.

A polybutadiene in which the proportion of 1,2-vinyl bonds is equal to or less than 2.0% by weight is preferred. The polybutadiene can contribute to the resilience performance of the core 4. In this respect, the proportion of 1,2-vinyl bonds is preferably equal to or less than 1.7% by weight and particularly preferably equal to or less than 1.5% by weight.

From the standpoint that a polybutadiene having a low proportion of 1,2-vinyl bonds and excellent polymerization activity is obtained, a polybutadiene synthesized with a rare-earth-element-containing catalyst is preferred. In particular, a polybutadiene synthesized with a catalyst containing neodymium, which is a lanthanum-series rare earth element compound, is preferred.

The polybutadiene has a Mooney viscosity (ML₁₊₄(100°C)) of preferably 30 or greater, more preferably 32 or greater, and particularly preferably 35 or greater. The Mooney viscosity (ML₁₊₄(100°C)) is preferably equal to or less than 140, more preferably equal to or less than 120, even more preferably equal to or less than 100, and particularly preferably equal to or less than 80. The Mooney viscosity (ML₁₊₄(100°C)) is measured according to the standards of "JIS K6300". The measurement conditions are as follows.
Rotor: L rotor
Preheating time: 1 minute
Rotating time of rotor: 4 minutes
Temperature: 100°C

In light of workability, the polybutadiene has a molecular weight distribution (Mw/Mn) of preferably 2.0 or greater, more preferably 2.2 or greater, even more preferably 2.4 or greater, and particularly preferably 2.6 or greater. In light of resilience performance, the molecular weight distribution (Mw/Mn) is preferably equal to or less than 6.0, more preferably equal to or less than 5.0, even more preferably equal to or less than 4.0, and particularly preferably equal to or less than 3.4. The molecular weight distribution (Mw/Mn) is calculated by dividing the weight average molecular weight Mw by the number average molecular weight Mn.

The molecular weight distribution is measured by gel permeation chromatography ("HLC-8120GPC" manufactured by Tosoh Corporation). The measurement conditions are as follows.
Detector: differential refractometer
Column: GMHHXL (manufactured by Tosoh Corporation)
Column temperature: 40°C
Mobile phase: tetrahydrofuran
The molecular weight distribution is calculated as a value obtained by conversion using polystyrene standard.

The co-crosslinking agent (b) is:
(b1) an α,β-unsaturated carboxylic acid having 3 to 8 carbon atoms; and/or
(b2) a metal salt of an α,β-unsaturated carboxylic acid having 3 to 8 carbon atoms.

The rubber composition may include only the α,β-unsaturated carboxylic acid (b1) or only the metal salt (b2) of the α,β-unsaturated carboxylic acid as the co-crosslinking agent (b). The rubber composition may include both the α,β-unsaturated carboxylic acid (b1) and the metal salt (b2) of the α,β-unsaturated carboxylic acid as the co-crosslinking agent (b).

The metal salt (b2) of the α,β-unsaturated carboxylic acid graft-polymerizes with the molecular chain of the base rubber, thereby crosslinking the rubber molecules. When the rubber composition includes the α,β-unsaturated carboxylic acid (b1), the rubber composition preferably further includes a metal compound (e). The metal compound (e) reacts with the α,β-unsaturated carboxylic acid (b1) in the rubber composition. A salt obtained by this reaction graft-polymerizes with the molecular chain of the base rubber.

Examples of the metal compound (e) include metal hydroxides such as magnesium hydroxide, zinc hydroxide, calcium hydroxide, sodium hydroxide, lithium hydroxide, potassium hydroxide, and copper hydroxide; metal oxides such as magnesium oxide, calcium oxide, zinc oxide, and copper oxide; and metal carbonates such as magnesium carbonate, zinc carbonate, calcium carbonate, sodium carbonate, lithium carbonate, and potassium carbonate. A compound that includes a bivalent metal is preferred. The compound that includes the bivalent metal reacts with the co-crosslinking agent (b) to form metal crosslinks. The metal compound (e) is particularly preferably a zinc compound. Two or more metal compounds may be used in combination.

Examples of the α,β-unsaturated carboxylic acid (b1) include acrylic acid, methacrylic acid, fumaric acid, maleic acid, and crotonic acid. Examples of the metal component in the metal salt (b2) of the α,β-unsaturated carboxylic acid include sodium ion, potassium ion, lithium ion, magnesium ion, calcium ion, zinc ion, barium ion, cadmium ion, aluminum ion, tin ion, and zirconium ion. The metal salt (b2) of the α,β-unsaturated carboxylic acid may include two or more types of ions. From the standpoint that metal crosslinks are likely to occur between the rubber molecules, bivalent metal ions such as magnesium ion, calcium ion, zinc ion, barium ion, and cadmium ion are preferred. The metal salt (b2) of the α,β-unsaturated carboxylic acid is particularly preferably zinc acrylate.

In light of resilience performance of the golf ball 2, the amount of the co-crosslinking agent (b) is preferably equal to or greater than 15 parts by weight and particularly preferably equal to or greater than 20 parts by weight, per 100 parts by weight of the base rubber. In light of feel at impact, the amount is preferably equal to or less than 50 parts by weight, more preferably equal to or less than 45 parts by weight, and particularly preferably equal to or less than 40 parts by weight, per 100 parts by weight of the base rubber.

The crosslinking initiator (c) is preferably an organic peroxide. The organic peroxide contributes to the resilience performance of the golf ball 2. Examples of preferable organic peroxides include dicumyl peroxide, 1,1-bis(t-butylperoxy)-3,3,5-trimethylcyclohexane, 2,5-dimethyl-2,5-di(t-butylperoxy)hexane, and di-t-butyl peroxide. In light of versatility, dicumyl peroxide is preferred.

In light of resilience performance of the golf ball 2, the amount of the crosslinking initiator (c) is preferably equal to or greater than 0.2 parts by weight and particularly preferably equal to or greater than 0.5 parts by weight, per 100 parts by weight of the base rubber. In light of feel at impact and durability of the golf ball 2, the amount is preferably equal to or less than 5 parts by weight and particularly preferably equal to or less than 2.5 parts by weight, per 100 parts by weight of the base rubber.

The acid component included in the acid and/or the salt (d) has reactivity with a cationic component. During heating and forming of the core 4, the acid dissociates and reacts with the cationic component of the co-crosslinking agent (b). It is thought that the acid inhibits formation of the metal crosslinks by the co-crosslinking agent (b) in the central portion of the core 4. The acid component included in the salt exchanges the cationic component with the co-crosslinking agent (b). It is inferred that during heating and forming of the core 4, the salt breaks the metal crosslinks by the co-crosslinking agent (b) in the central portion of the core 4.

Examples of the acid and/or the salt (d) include oxo acids, such as carboxylic acids, sulfonic acids, and phosphoric acid, and salts thereof; and hydroacids, such as hydrochloric acid and hydrofluoric acid, and salts thereof. Oxo acids and salts thereof are preferred. In light of affinity with the base rubber, the acid and/or the salt (d) is preferably a carboxylic acid and/or a salt thereof (d1). In the present invention, the co-crosslinking agent (b) is not included in the concept of the acid and/or the salt (d).

In light of reactivity with the co-crosslinking agent (b), the carbon number of the carboxylic acid component of the carboxylic acid and/or the salt thereof (d1) is preferably equal to or greater than 1 and more preferably equal to or greater than 5. The carbon number of the carboxylic acid component of the carboxylic acid and/or the salt thereof (d1) is preferably equal to or less than 30 and particularly preferably equal to or less than 20. Examples of preferable carboxylic acids and/or salts thereof (d1) include aliphatic carboxylic acids (fatty acids) and salts thereof, and aromatic carboxylic acids and salts thereof. In light of affinity with the base rubber, fatty acids and salts thereof are preferred.

The rubber composition may include a saturated fatty acid and a salt thereof or may include an unsaturated fatty acid and a salt thereof. The saturated fatty acid and the salt thereof are more preferred.

Examples of fatty acids include butyric acid (C4), valeric acid (C5), caproic acid (C6), enanthic acid (C7), caprylic acid (octanoic acid) (C8), pelargonic acid (C9), capric acid (decanoic acid) (C10), lauric acid (C12), myristic acid (C14), myristoleic acid (C14), pentadecylic acid (C15), palmitic acid (C16), palmitoleic acid (C16), margaric acid (C17), stearic acid (C18), elaidic acid (C18), vaccenic acid (C18), oleic acid (C18), linolic acid (C18), linolenic acid (C18), 12-hydroxystearic acid (C18), arachidic acid (C20), gadoleic acid (C20), arachidonic acid (C20), eicosenoic acid (C20), behenic acid (C22), erucic acid (C22), lignoceric acid (C24), nervonic acid (C24), cerotic acid (C26), montanic acid (C28), and melissic acid (C30) . Two or more fatty acids may be used in combination. Caprylic acid (octanoic acid), lauric acid, myristic acid, palmitic acid, stearic acid, oleic acid, and behenic acid are preferred.

An aromatic carboxylic acid has an aromatic ring and a carboxyl group. Examples of aromatic carboxylic acids include benzoic acid, phthalic acid, isophthalic acid, terephthalic acid, hemimellitic acid (benzene-1,2,3-tricarboxylic acid), trimellitic acid (benzene-1,2,4-tricarboxylic acid), trimesic acid (benzene-1,3,5-tricarboxylic acid), mellophanic acid (benzene-1,2,3,4-tetracarboxylic acid), prehnitic acid (benzene-1,2,3,5-tetracarboxylic acid), pyromellitic acid (benzene-1,2,4,5-tetracarboxylicacid), melliticacid (benzene hexacarboxylic acid), diphenic acid (biphenyl-2,2'-dicarboxylic acid), toluic acid (methylbenzoic acid), xylic acid, prehnitylic acid (2,3,4-trimethylbenzoic acid), γ-isodurylic acid (2,3,5-trimethylbenzoic acid), durylic acid (2,4,5-trimethylbenzoic acid), β-isodurylic acid (2,4,6-trimethylbenzoic acid), α-isodurylic acid (3,4,5-trimethylbenzoic acid), cuminic acid (4-isopropylbenzoic acid), uvitic acid (5-methylisophthalic acid), α-toluic acid (phenylacetic acid), hydratropic acid (2-phenylpropanoic acid), and hydrocinnamic acid (3-phenylpropanoic acid).

The rubber composition may include an aromatic carboxylic acid substituted with a hydroxyl group, an alkoxy group, or an oxo group. Specific examples of this carboxylic acid can include salicylic acid (2-hydroxybenzoic acid), anisic acid (methoxybenzoic acid), cresotinic acid (hydroxy(methyl) benzoic acid), o-homosalicylicacid (2-hydroxy-3-methylbenzoic acid), m-homosalicylic acid (2-hydroxy-4-methylbenzoic acid), p-homosalicylic acid (2-hydroxy-5-methylbenzoic acid), o-pyrocatechuic acid (2,3-dihydroxybenzoic acid), β-resorcylic acid (2,4-dihydroxybenzoic acid), γ-resorcylic acid (2,6-dihydroxybenzoic acid), protocatechuic acid (3,4-dihydroxybenzoic acid), α-resorcylic acid (3,5-dihydroxybenzoic acid), vanillic acid (4-hydroxy-3-methoxybenzoic acid), isovanillic acid (3-hydroxy-4-methoxybenzoic acid), veratric acid (3,4-dimethoxybenzoic acid), o-veratric acid (2,3-dimethoxybenzoic acid), orsellinic acid (2,4-dihydroxy-6-methylbenzoic acid), m-hemipinic acid (4,5-dimethoxyphthalic acid), gallic acid (3,4,5-trihydroxybenzoic acid), syringic acid (4-hydroxy-3,5-dimethoxybenzoic acid), asaronic acid (2,4,5-trimethoxybenzoic acid), mandelic acid (hydroxy(phenyl)acetic acid), vanillylmandelic acid (hydroxy(4-hydroxy-3-methoxyphenyl)acetic acid), homoanisic acid ((4-methoxyphenyl)acetic acid), homogentisic acid ((2,5-dihydroxyphenyl)acetic acid), homoprotocatechuic acid ((3,4-dihydroxyphenyl)acetic acid), homovanillic acid ((4-hydroxy-3-methoxyphenyl)acetic acid), homoisovanillic acid ((3-hydroxy-4-methoxyphenyl)acetic acid), homoveratric acid ((3,4-dimethoxyphenyl)acetic acid), o-homoveratric acid ((2,3-dimethoxyphenyl)acetic acid), homophthalic acid (2-(carboxymethyl)benzoic acid), homoisophthalic acid (3-(carboxymethyl)benzoic acid), homoterephthalic acid (4-(carboxymethyl)benzoic acid), phthalonic acid (2-(carboxycarbonyl)benzoic acid), isophthalonic acid (3-(carboxycarbonyl)benzoic acid), terephthalonic acid (4-(carboxycarbonyl)benzoic acid), benzilic acid (hydroxydiphenylacetic acid), atrolactic acid (2-hydroxy-2-phenylpropanoic acid), tropic acid (3-hydroxy-2-phenylpropanoic acid), melilotic acid (3-(2-hydroxyphenyl)propanoic acid), phloretic acid (3-(4-hydroxyphenyl)propanoic acid), hydrocaffeic acid (3-(3,4-dihydroxyphenyl)propanoic acid), hydroferulic acid (3-(4-hydroxy-3-methoxyphenyl)propanoic acid), hydroisoferulic acid (3-(3-hydroxy-4-methoxyphenyl)propanoic acid), p-coumaric acid (3-(4-hydroxyphenyl)acrylic acid), umbellic acid (3-(2,4-dihydroxyphenyl)acrylic acid), caffeic acid (3-(3,4-dihydroxyphenyl)acrylic acid), ferulic acid (3-(4-hydroxy-3-methoxyphenyl)acrylic acid), isoferulic acid (3-(3-hydroxy-4-methoxyphenyl)acrylic acid), and sinapic acid (3-(4-hydroxy-3,5-dimethoxyphenyl)acrylic acid).

The cationic component included in the acid and/or the salt (d) is a metal ion or an organic cation. Examples of the metal ion include sodium ion, potassium ion, lithium ion, silver ion, magnesium ion, calcium ion, zinc ion, barium ion, cadmium ion, copper ion, cobalt ion, nickel ion, manganese ion, aluminum ion, iron ion, tin ion, zirconium ion, and titanium ion. Two or more types of ions may be used in combination. Zinc ion and magnesium ion are preferred.

The organic cation is a cation having a carbon chain. Examples of the organic cation include organic ammonium ions. Examples of organic ammonium ions include primary ammonium ions such as stearylammonium ion, hexylammonium ion, octylammonium ion, and 2-ethylhexylammonium ion; secondary ammonium ions such as dodecyl(lauryl)ammonium ion, and octadecyl(stearyl)ammonium ion; tertiary ammonium ions such as trioctylammonium ion; and quaternary ammonium ions such as dioctyldimethylammonium ion, and distearyldimethylammonium ion. Two or more types of organic cations may be used in combination.

In light of ease of the above cation exchange reaction, a salt of a fatty acid is particularly preferred. A fatty acid and a salt of a fatty acid may be used in combination, and salts of two or more fatty acids may be used in combination.

Examples of preferable salts of carboxylic acids include potassium salts, magnesium salts, aluminum salts, zinc salts, iron salts, copper salts, nickel salts, and cobalt salts of octanoic acid, lauric acid, myristic acid, palmitic acid, stearic acid, oleic acid, and behenic acid. Zinc salts of carboxylic acids are particularly preferred. Examples of particularly preferable salts of carboxylic acids include zinc octoate, zinc laurate, zinc myristate, and zinc stearate.

From the standpoint that a hardness distribution of the core 4 is made appropriate, the amount of the acid and/or the salt (d) is preferably equal to or greater than 0.5 parts by weight, more preferably equal to or greater than 1.0 parts by weight, even more preferably equal to or greater than 1.5 parts by weight, and further preferably equal to or greater than 2 parts by weight, per 100 parts by weight of the base rubber. In light of resilience performance, the amount is preferably equal to or less than 45 parts by weight, more preferably equal to or less than 40 parts by weight, and particularly preferably equal to or less than 30 parts by weight, per 100 parts by weight of the base rubber.

The weight ratio of the co-crosslinking agent (b) and the acid and/or the salt (d) in the rubber composition is preferably equal to or greater than 3/7 but equal to or less than 9/1, and is particularly preferably equal to or greater than 4/6 but equal to or less than 8/2. From the rubber composition in which this weight ratio is within the above range, the core 4 whose hardness linearly increases from its central point toward its surface is obtained.

As the co-crosslinking agent (b), zinc acrylate is preferably used. Zinc acrylate whose surface is coated with stearic acid or zinc stearate for the purpose of improving dispersibility to rubber is present. When the rubber composition includes this zinc acrylate, the stearic acid or zinc stearate coating the zinc acrylate is not included in the concept of the acid and/or the salt (d).

The rubber composition preferably further includes an organic sulfur compound (f). The organic sulfur compound (f) can contribute to control of: the linearity of the hardness distribution of the core 4; and the degree of an outer-hard/inner-soft structure. An example of the organic sulfur compound (f) is an organic compound having a thiol group or a polysulfide linkage having 2 to 4 sulfur atoms. A metal salt of this organic compound is also included in the organic sulfur compound (f). Examples of the organic sulfur compound (f) include aliphatic compounds such as aliphatic thiols, aliphatic thiocarboxylic acids, aliphatic dithiocarboxylic acids, and aliphatic polysulfides; heterocyclic compounds; alicyclic compounds such as alicyclic thiols, alicyclic thiocarboxylic acids, alicyclic dithiocarboxylic acids, and alicyclic polysulfides; and aromatic compounds. Specific examples of the organic sulfur compound (f) include thiophenols, thionaphthols, polysulfides, thiocarboxylic acids, dithiocarboxylic acids, sulfenamides, thiurams, dithiocarbamates, and thiazoles. Preferable organic sulfur compounds (e) are thiophenols, diphenyl disulfides, thionaphthols, thiuram disulfides, and metal salts thereof.

Specific examples of the organic sulfur compound (f) are represented by the following chemical formulas (1) to (4).

In the chemical formula (1), R1 to R5 each represent H or a substituent.

In the chemical formula (2), R1 to R10 each represent H or a substituent.

In the chemical formula (3), R1 to R5 each represent H or a substituent, and M1 represents a monovalent metal atom.

In the chemical formula (4), R1 to R10 each represent H or a substituent, and M2 represents a bivalent metal atom.

In the formulas (1) to (4), each substituent is at least one group selected from the group consisting of a halogen group (F, Cl, Br, I), an alkyl group, a carboxyl group (-COOH), an ester (-COOR) of a carboxyl group, a formyl group (-CHO), an acyl group (-COR), a carbonyl halide group (-COX), a sulfo group (-SO₃H), an ester (-SO₃R) of a sulfo group, a sulfonyl halide group (-SO₂X), a sulfino group (-SO₂H), an alkylsulfinyl group (-SOR), a carbamoyl group (-CONH₂), an alkyl halide group, a cyano group (-CN), and an alkoxy group (-OR).

Examples of the organic sulfur compound represented by the chemical formula (1) include thiophenol; thiophenols substituted with halogen groups, such as 4-fluorothiophenol, 2,5-difluorothiophenol, 2,4,5-trifluorothiophenol, 2,4,5,6-tetrafluorothiophenol, pentafluorothiophenol, 2-chlorothiophenol, 4-chlorothiophenol, 2,4-dichlorothiophenol, 2,5-dichlorothiophenol, 2,6-dichlorothiophenol, 2,4,5-trichlorothiophenol, 2,4,5,6-tetrachlorothiophenol, pentachlorothiophenol, 4-bromothiophenol, 2,5-dibromothiophenol, 2,4,5-tribromothiophenol, 2,4,5,6-tetrabromothiophenol, pentabromothiophenol, 4-iodothiophenol, 2,5-diiodothiophenol, 2,4,5-triiodothiophenol, 2,4,5,6-tetraiodothiophenol, and pentaiodothiophenol; thiophenols substituted with alkyl groups, such as 4-methylthiophenol, 2,4,5-trimethylthiophenol, pentamethylthiophenol, 4-t-butylthiophenol, 2,4,5-tri-t-butylthiophenol, and penta-t-butylthiophenol; thiophenols substituted with carboxyl groups, such as 4-carboxythiophenol, 2,4,6-tricarboxythiophenol, and pentacarboxythiophenol; thiophenols substituted with alkoxycarbonyl groups, such as 4-methoxycarbonylthiophenol, 2,4,6-trimethoxycarbonylthiophenol, and pentamethoxycarbonylthiophenol; thiophenols substituted with formyl groups, such as 4-formylthiophenol, 2,4,6-triformylthiophenol, and pentaformylthiophenol; thiophenols substituted with acyl groups, such as 4-acetylthiophenol, 2,4,6-triacetylthiophenol, and pentaacetylthiophenol; thiophenols substituted with carbonyl halide groups, such as 4-chlorocarbonylthiophenol, 2,4,6-tri(chlorocarbonyl)thiophenol, and penta(chlorocarbonyl)thiophenol; thiophenols substituted with sulfo groups, such as 4-sulfothiophenol, 2,4,6-trisulfothiophenol, and pentasulfothiophenol; thiophenols substituted with alkoxysulfonyl groups, such as 4-methoxysulfonylthiophenol, 2,4,6-trimethoxysulfonylthiophenol, and pentamethoxysulfonylthiophenol; thiophenols substituted with sulfonyl halide groups, such as 4-chlorosulfonylthiophenol, 2,4,6-tri(chlorosulfonyl)thiophenol, and penta(chlorosulfonyl)thiophenol; thiophenols substituted with sulfino groups, such as 4-sulfinothiophenol, 2,4,6-trisulfinothiophenol, and pentasulfinothiophenol; thiophenols substituted with alkylsulfinyl groups, such as 4-methylsulfinylthiophenol, 2,4,6-tri(methylsulfinyl)thiophenol, and penta (methylsulfinyl)thiophenol; thiophenols substituted with carbamoyl groups, such as 4-carbamoylthiophenol, 2,4,6-tricarbamoylthiophenol, and pentacarbamoylthiophenol; thiophenols substituted with alkyl halide groups, such as 4-trichloromethylthiophenol, 2,4,6-tri(trichloromethyl)thiophenol, and penta(trichloromethyl)thiophenol; thiophenols substituted with cyano groups, such as 4-cyanothiophenol, 2,4,6-tricyanothiophenol, and pentacyanothiophenol; and thiophenols substituted with alkoxy groups, such as 4-methoxythiophenol, 2,4,6-trimethoxythiophenol, and pentamethoxythiophenol. Each of these thiophenols is substituted with one type of substituent.

Another example of the organic sulfur compound represented by the chemical formula (1) is a compound substituted with at least one type of the above substituents and another substituent. Examples of the other substituent include a nitro group (-NO₂), an amino group (-NH₂), a hydroxyl group (-OH), and a phenylthio group (-SPh). Specific examples of the compound include 4-chloro-2-nitrothiophenol, 4-chloro-2-aminothiophenol, 4-chloro-2-hydroxythiophenol, 4-chloro-2-phenylthiothiophenol, 4-methyl-2-nitrothiophenol, 4-methyl-2-aminothiophenol, 4-methyl-2-hydroxythiophenol, 4-methyl-2-phenylthiothiophenol, 4-carboxy-2-nitrothiophenol, 4-carboxy-2-aminothiophenol, 4-carboxy-2-hydroxythiophenol, 4-carboxy-2-phenylthiothiophenol, 4-methoxycarbonyl-2-nitrothiophenol, 4-methoxycarbonyl-2-aminothiophenol, 4-methoxycarbonyl-2-hydroxythiophenol, 4-methoxycarbonyl-2-phenylthiothiophenol, 4-formyl-2-nitrothiophenol, 4-formyl-2-aminothiophenol, 4-formyl-2-hydroxythiophenol, 4-formyl-2-phenylthiothiophenol, 4-acetyl-2-nitrothiophenol, 4-acetyl-2-aminothiophenol, 4-acetyl-2-hydroxythiophenol, 4-acetyl-2-phenylthiothiophenol, 4-chlorocarbonyl-2-nitrothiophenol, 4-chlorocarbonyl-2-aminothiophenol, 4-chlorocarbonyl-2-hydroxythiophenol, 4-chlorocarbonyl-2-phenylthiothiophenol, 4-sulfo-2-nitrothiophenol, 4-sulfo-2-aminothiophenol, 4-sulfo-2-hydroxythiophenol, 4-sulfo-2-phenylthiothiophenol, 4-methoxysulfonyl-2-nitrothiophenol, 4-methoxysulfonyl-2-aminothiophenol, 4-methoxysulfonyl-2-hydroxythiophenol, 4-methoxysulfonyl-2-phenylthiothiophenol, 4-chlorosulfonyl-2-nitrothiophenol, 4-chlorosulfonyl-2-aminothiophenol, 4-chlorosulfonyl-2-hydroxythiophenol, 4-chlorosulfonyl-2-phenylthiothiophenol, 4-sulfino-2-nitrothiophenol, 4-sulfino-2-aminothiophenol, 4-sulfino-2-hydroxythiophenol, 4-sulfino-2-phenylthiothiophenol, 4-methylsulfinyl-2-nitrothiophenol, 4-methylsulfinyl-2-aminothiophenol, 4-methylsulfinyl-2-hydroxythiophenol, 4-methylsulfinyl-2-phenylthiothiophenol, 4-carbamoyl-2-nitrothiophenol, 4-carbamoyl-2-aminothiophenol, 4-carbamoyl-2-hydroxythiophenol, 4-carbamoyl-2-phenylthiothiophenol, 4-trichloromethyl-2-nitrothiophenol, 4-trichloromethyl-2-aminothiophenol, 4-trichloromethyl-2-hydroxythiophenol, 4-trichloromethyl-2-phenylthiothiophenol, 4-cyano-2-nitrothiophenol, 4-cyano-2-aminothiophenol, 4-cyano-2-hydroxythiophenol, 4-cyano-2-phenylthiothiophenol, 4-methoxy-2-nitrothiophenol, 4-methoxy-2-aminothiophenol, 4-methoxy-2-hydroxythiophenol, and 4-methoxy-2-phenylthiothiophenol.

Still another example of the organic sulfur compound represented by the chemical formula (1) is a compound substituted with two or more types of substituents. Specific examples of the compound include 4-acetyl-2-chlorothiophenol, 4-acetyl-2-methylthiophenol, 4-acetyl-2-carboxythiophenol, 4-acetyl-2-methoxycarbonylthiophenol, 4-acetyl-2-formylthiophenol, 4-acetyl-2-chlorocarbonylthiophenol, 4-acetyl-2-sulfothiophenol, 4-acetyl-2-methoxysulfonylthiophenol, 4-acetyl-2-chlorosulfonylthiophenol, 4-acetyl-2-sulfinothiophenol, 4-acetyl-2-methylsulfinylthiophenol, 4-acetyl-2-carbamoylthiophenol, 4-acetyl-2-trichloromethylthiophenol, 4-acetyl-2-cyanothiophenol, and 4-acetyl-2-methoxythiophenol.

Examples of the organic sulfur compound represented by the chemical formula (2) include diphenyl disulfide; diphenyl disulfides substituted with halogen groups, such as bis(4-fluorophenyl)disulfide, bis(2,5-difluorophenyl)disulfide, bis(2,4,5-trifluorophenyl)disulfide, bis(2,4,5,6-tetrafluorophenyl)disulfide, bis(pentafluorophenyl)disulfide, bis(4-chlorophenyl)disulfide, bis(2,5-dichlorophenyl)disulfide, bis(2,4,5-trichlorophenyl)disulfide, bis(2,4,5,6-tetrachlorophenyl)disulfide, bis(pentachlorophenyl)disulfide, bis(4-bromophenyl)disulfide, bis(2,5-dibromophenyl)disulfide, bis(2,4,5-tribromophenyl)disulfide, bis(2,4,5,6-tetrabromophenyl)disulfide, bis(pentabromophenyl)disulfide, bis(4-iodophenyl)disulfide, bis(2,5-diiodophenyl)disulfide, bis(2,4,5-triiodophenyl)disulfide, bis(2,4,5,6-tetraiodophenyl)disulfide, and bis(pentaiodophenyl)disulfide; diphenyl disulfides substituted with alkyl groups, such as bis(4-methylphenyl)disulfide, bis(2,4,5-trimethylphenyl)disulfide, bis(pentamethylphenyl)disulfide, bis(4-t-butylphenyl)disulfide, bis(2,4,5-tri-t-butylphenyl)disulfide, and bis(penta-t-butylphenyl)disulfide; diphenyl disulfides substituted with carboxyl groups, such as bis(4-carboxyphenyl)disulfide, bis(2,4,6-tricarboxyphenyl)disulfide, and bis(pentacarboxyphenyl)disulfide; diphenyl disulfides substituted with alkoxycarbonyl groups, such as bis(4-methoxycarbonylphenyl)disulfide, bis(2,4,6-trimethoxycarbonylphenyl)disulfide, and bis(pentamethoxycarbonylphenyl)disulfide; diphenyl disulfides substituted with formyl groups, such as bis(4-formylphenyl)disulfide, bis(2,4,6-triformylphenyl)disulfide, and bis(pentaformylphenyl)disulfide; diphenyl disulfides substituted with acyl groups, such as bis(4-acetylphenyl)disulfide, bis(2,4,6-triacetylphenyl)disulfide, and bis(pentaacetylphenyl)disulfide; diphenyl disulfides substituted with carbonyl halide groups, such as bis(4-chlorocarbonylphenyl)disulfide, bis(2,4,6-tri(chlorocarbonyl)phenyl)disulfide, and bis(penta(chlorocarbonyl)phenyl)disulfide; diphenyl disulfides substituted with sulfo groups, such as bis(4-sulfophenyl)disulfide, bis(2,4,6-trisulfophenyl)disulfide, and bis(pentasulfophenyl)disulfide; diphenyl disulfides substituted with alkoxysulfonyl groups, such as bis(4-methoxysulfonylphenyl)disulfide, bis(2,4,6-trimethoxysulfonylphenyl)disulfide, and bis(pentamethoxysulfonylphenyl)disulfide; diphenyl disulfides substituted with sulfonyl halide groups, such as bis(4-chlorosulfonylphenyl)disulfide, bis(2,4,6-tri(chlorosulfonyl)phenyl)disulfide, and bis(penta(chlorosulfonyl)phenyl)disulfide; diphenyl disulfides substituted with sulfino groups, such as bis(4-sulfinophenyl)disulfide, bis(2,4,6-trisulfinophenyl)disulfide, and bis(pentasulfinophenyl)disulfide; diphenyl disulfides substituted with alkylsulfinyl groups, such as bis(4-methylsulfinylphenyl)disulfide, bis(2,4,6-tri(methylsulfinyl)phenyl)disulfide, and bis(penta(methylsulfinyl)phenyl)disulfide; diphenyl disulfides substituted with carbamoyl groups, such as bis(4-carbamoylphenyl)disulfide, bis(2,4,6-tricarbamoylphenyl)disulfide, and bis(pentacarbamoylphenyl)disulfide; diphenyl disulfides substituted with alkyl halide groups, such as bis(4-trichloromethylphenyl)disulfide, bis(2,4,6-tri(trichloromethyl)phenyl)disulfide, and bis(penta(trichloromethyl)phenyl)disulfide; diphenyl disulfides substituted with cyano groups, such as bis(4-cyanophenyl)disulfide, bis(2,4,6-tricyanophenyl)disulfide, and bis(pentacyanophenyl)disulfide; and diphenyl disulfides substituted with alkoxy groups, such as bis(4-methoxyphenyl)disulfide, bis(2,4,6-trimethoxyphenyl)disulfide, and bis(pentamethoxyphenyl)disulfide. Each of these diphenyl disulfides is substituted with one type of substituent.

Another example of the organic sulfur compound represented by the chemical formula (2) is a compound substituted with at least one type of the above substituents and another substituent. Examples of the other substituent include a nitro group (-NO₂), an amino group (-NH₂), a hydroxyl group (-OH), and a phenylthio group (-SPh). Specific examples of the compound include bis(4-chloro-2-nitrophenyl)disulfide, bis(4-chloro-2-aminophenyl)disulfide, bis(4-chloro-2-hydroxyphenyl)disulfide, bis(4-chloro-2-phenylthiophenyl)disulfide, bis(4-methyl-2-nitrophenyl)disulfide, bis(4-methyl-2-aminophenyl)disulfide, bis(4-methyl-2-hydroxyphenyl)disulfide, bis(4-methyl-2-phenylthiophenyl)disulfide, bis(4-carboxy-2-nitrophenyl)disulfide, bis(4-carboxy-2-aminophenyl)disulfide, bis(4-carboxy-2-hydroxyphenyl)disulfide, bis(4-carboxy-2-phenylthiophenyl)disulfide, bis(4-methoxycarbonyl-2-nitrophenyl)disulfide, bis(4-methoxycarbonyl-2-aminophenyl)disulfide, bis(4-methoxycarbonyl-2-hydroxyphenyl)disulfide, bis(4-methoxycarbonyl-2-phenylthiophenyl)disulfide, bis(4-formyl-2-nitrophenyl)disulfide, bis(4-formyl-2-aminophenyl)disulfide, bis(4-formyl-2-hydroxyphenyl)disulfide, bis(4-formyl-2-phenylthiophenyl)disulfide, bis(4-acetyl-2-nitrophenyl)disulfide, bis(4-acetyl-2-aminophenyl)disulfide, bis(4-acetyl-2-hydroxyphenyl)disulfide, bis(4-acetyl-2-phenylthiophenyl)disulfide, bis(4-chlorocarbonyl-2-nitrophenyl)disulfide, bis(4-chlorocarbonyl-2-aminophenyl)disulfide, bis(4-chlorocarbonyl-2-hydroxyphenyl)disulfide, bis(4-chlorocarbonyl-2-phenylthiophenyl)disulfide, bis(4-sulfo-2-nitrophenyl)disulfide, bis(4-sulfo-2-aminophenyl)disulfide, bis(4-sulfo-2-hydroxyphenyl)disulfide, bis(4-sulfo-2-phenylthiophenyl)disulfide, bis(4-methoxysulfonyl-2-nitrophenyl)disulfide, bis(4-methoxysulfonyl-2-aminophenyl)disulfide, bis(4-methoxysulfonyl-2-hydroxyphenyl)disulfide, bis(4-methoxysulfonyl-2-phenylthiophenyl)disulfide, bis(4-chlorosulfonyl-2-nitrophenyl)disulfide, bis(4-chlorosulfonyl-2-aminophenyl)disulfide, bis(4-chlorosulfonyl-2-hydroxyphenyl)disulfide, bis(4-chlorosulfonyl-2-phenylthiophenyl)disulfide, bis(4-sulfino-2-nitrophenyl)disulfide, bis(4-sulfino-2-aminophenyl)disulfide, bis(4-sulfino-2-hydroxyphenyl)disulfide, bis(4-sulfino-2-phenylthiophenyl)disulfide, bis(4-methylsulfinyl-2-nitrophenyl)disulfide, bis(4-methylsulfinyl-2-aminophenyl)disulfide, bis(4-methylsulfinyl-2-hydroxyphenyl)disulfide, bis(4-methylsulfinyl-2-phenylthiophenyl)disulfide, bis(4-carbamoyl-2-nitrophenyl)disulfide, bis(4-carbamoyl-2-aminophenyl)disulfide, bis(4-carbamoyl-2-hydroxyphenyl)disulfide, bis(4-carbamoyl-2-phenylthiophenyl)disulfide, bis(4-trichloromethyl-2-nitrophenyl)disulfide, bis(4-trichloromethyl-2-aminophenyl)disulfide, bis(4-trichloromethyl-2-hydroxyphenyl)disulfide, bis(4-trichloromethyl-2-phenylthiophenyl)disulfide, bis(4-cyano-2-nitrophenyl)disulfide, bis(4-cyano-2-aminophenyl)disulfide, bis(4-cyano-2-hydroxyphenyl)disulfide, bis(4-cyano-2-phenylthiophenyl)disulfide, bis(4-methoxy-2-nitrophenyl)disulfide, bis(4-methoxy-2-aminophenyl)disulfide, bis(4-methoxy-2-hydroxyphenyl)disulfide, and bis(4-methoxy-2-phenylthiophenyl)disulfide.

Still another example of the organic sulfur compound represented by the chemical formula (2) is a compound substituted with two or more types of substituents. Specific examples of the compound include bis(4-acetyl-2-chlorophenyl)disulfide, bis(4-acetyl-2-methylphenyl)disulfide, bis(4-acetyl-2-carboxyphenyl)disulfide, bis(4-acetyl-2-methoxycarbonylphenyl)disulfide, bis(4-acetyl-2-formylphenyl)disulfide, bis(4-acetyl-2-chlorocarbonylphenyl)disulfide, bis(4-acetyl-2-sulfophenyl)disulfide, bis(4-acetyl-2-methoxysulfonylphenyl)disulfide, bis(4-acetyl-2-chlorosulfonylphenyl)disulfide, bis(4-acetyl-2-sulfinophenyl)disulfide, bis(4-acetyl-2-methylsulfinylphenyl)disulfide, bis(4-acetyl-2-carbamoylphenyl)disulfide, bis(4-acetyl-2-trichloromethylphenyl)disulfide, bis(4-acetyl-2-cyanophenyl)disulfide, and bis(4-acetyl-2-methoxyphenyl)disulfide.

Examples of the organic sulfur compound represented by the chemical formula (3) include thiophenol sodium salt; thiophenol sodium salts substituted with halogen groups, such as 4-fluorothiophenol sodium salt, 2,5-difluorothiophenol sodium salt, 2,4,5-trifluorothiophenol sodium salt, 2,4,5,6-tetrafluorothiophenol sodium salt, pentafluorothiophenol sodium salt, 4-chlorothiophenol sodium salt, 2,5-dichlorothiophenol sodium salt, 2,4,5-trichlorothiophenol sodium salt, 2,4,5,6-tetrachlorothiophenol sodium salt, pentachlorothiophenol sodium salt, 4-bromothiophenol sodium salt, 2,5-dibromothiophenol sodium salt, 2,4,5-tribromothiophenol sodium salt, 2,4,5,6-tetrabromothiophenol sodium salt, pentabromothiophenol sodium salt, 4-iodothiophenol sodium salt, 2,5-diiodothiophenol sodium salt, 2,4,5-triiodothiophenol sodium salt, 2,4,5,6-tetraiodothiophenol sodium salt, and pentaiodothiophenol sodium salt; thiophenol sodium salts substituted with alkyl groups, such as 4-methylthiophenol sodium salt, 2,4,5-trimethylthiophenol sodium salt, pentamethylthiophenol sodium salt, 4-t-butylthiophenol sodium salt, 2,4,5-tri-t-butylthiophenol sodium salt, and penta(t-butyl)thiophenol sodium salt; thiophenol sodium salts substituted with carboxyl groups, such as 4-carboxythiophenol sodium salt, 2,4,6-tricarboxythiophenol sodium salt, and pentacarboxythiophenol sodium salt; thiophenol sodium salts substituted with alkoxycarbonyl groups, such as 4-methoxycarbonylthiophenol sodium salt, 2,4,6-trimethoxycarbonylthiophenol sodium salt, and pentamethoxycarbonylthiophenol sodium salt; thiophenol sodium salts substituted with formyl groups, such as 4-formylthiophenol sodium salt, 2,4,6-triformylthiophenol sodium salt, and pentaformylthiophenol sodium salt; thiophenol sodium salts substituted with acyl groups, such as 4-acetylthiophenol sodium salt, 2,4,6-triacetylthiophenol sodium salt, and pentaacetylthiophenol sodium salt; thiophenol sodium salts substituted with carbonyl halide groups, such as 4-chlorocarbonylthiophenol sodium salt, 2,4,6-tri(chlorocarbonyl)thiophenol sodium salt, and penta(chlorocarbonyl)thiophenol sodium salt; thiophenol sodium salts substituted with sulfo groups, such as 4-sulfothiophenol sodium salt, 2,4,6-trisulfothiophenol sodium salt, and pentasulfothiophenol sodium salt; thiophenol sodium salts substituted with alkoxysulfonyl groups, such as 4-methoxysulfonylthiophenol sodium salt, 2,4,6-trimethoxysulfonylthiophenol sodium salt, and pentamethoxysulfonylthiophenol sodium salt; thiophenol sodium salts substituted with sulfonyl halide groups, such as 4-chlorosulfonylthiophenol sodium salt, 2,4,6-tri(chlorosulfonyl)thiophenol sodium salt, and penta(chlorosulfonyl)thiophenolsodiumsalt;thiophenolsodium salts substituted with sulfino groups, such as 4-sulfinothiophenol sodium salt, 2,4,6-trisulfinothiophenol sodium salt, and pentasulfinothiophenol sodium salt; thiophenol sodium salts substituted with alkylsulfinyl groups, such as 4-methylsulfinylthiophenol sodium salt, 2,4,6-tri(methylsulfinyl)thiophenol sodium salt, and penta(methylsulfinyl)thiophenol sodium salt; thiophenol sodium salts substituted with carbamoyl groups, such as 4-carbamoylthiophenol sodium salt, 2,4,6-tricarbamoylthiophenol sodium salt, and pentacarbamoylthiophenol sodium salt; thiophenol sodium salts substituted with alkyl halide groups, such as 4-trichloromethylthiophenol sodium salt, 2,4,6-tri(trichloromethyl)thiophenol sodium salt, and penta(trichloromethyl)thiophenol sodium salt; thiophenol sodium salts substituted with cyano groups, such as 4-cyanothiophenolsodiumsalt, 2,4,6-tricyanothiophenolsodium salt, and pentacyanothiophenol sodium salt; and thiophenol sodium salts substituted with alkoxy groups, such as 4-methoxythiophenol sodium salt, 2,4,6-trimethoxythiophenol sodium salt, and pentamethoxythiophenol sodium salt. Each of these thiophenol sodium salts is substituted with one type of substituent.

Another example of the organic sulfur compound represented by the chemical formula (3) is a compound substituted with at least one type of the above substituents and another substituent. Examples of the other substituent include a nitro group (-NO₂), an amino group (-NH₂), a hydroxyl group (-OH), and a phenylthio group (-SPh). Specific examples of the compound include 4-chloro-2-nitrothiophenol sodium salt, 4-chloro-2-aminothiophenol sodium salt, 4-chloro-2-hydroxythiophenol sodium salt, 4-chloro-2-phenylthiothiophenol sodium salt, 4-methyl-2-nitrothiophenol sodium salt, 4-methyl-2-aminothiophenol sodium salt, 4-methyl-2-hydroxythiophenol sodium salt, 4-methyl-2-phenylthiothiophenol sodium salt, 4-carboxy-2-nitrothiophenol sodium salt, 4-carboxy-2-aminothiophenol sodium salt, 4-carboxy-2-hydroxythiophenol sodium salt, 4-carboxy-2-phenylthiothiophenol sodium salt, 4-methoxycarbonyl-2-nitrothiophenol sodium salt, 4-methoxycarbonyl-2-aminothiophenol sodium salt, 4-methoxycarbonyl-2-hydroxythiophenol sodium salt, 4-methoxycarbonyl-2-phenylthiothiophenol sodium salt, 4-formyl-2-nitrothiophenol sodium salt, 4-formyl-2-aminothiophenol sodium salt, 4-formyl-2-hydroxythiophenol sodium salt, 4-formyl-2-phenylthiothiophenol sodium salt, 4-acetyl-2-nitrothiophenol sodium salt, 4-acetyl-2-aminothiophenol sodium salt, 4-acetyl-2-hydroxythiophenol sodium salt, 4-acetyl-2-phenylthiothiophenol sodium salt, 4-chlorocarbonyl-2-nitrothiophenol sodium salt, 4-chlorocarbonyl-2-aminothiophenol sodium salt, 4-chlorocarbonyl-2-hydroxythiophenol sodium salt, 4-chlorocarbonyl-2-phenylthiothiophenol sodium salt, 4-sulfo-2-nitrothiophenol sodium salt, 4-sulfo-2-aminothiophenol sodium salt, 4-sulfo-2-hydroxythiophenol sodium salt, 4-sulfo-2-phenylthiothiophenol sodium salt, 4-methoxysulfonyl-2-nitrothiophenol sodium salt, 4-methoxysulfonyl-2-aminothiophenol sodium salt, 4-methoxysulfonyl-2-hydroxythiophenol sodium salt, 4-methoxysulfonyl-2-phenylthiothiophenol sodium salt, 4-chlorosulfonyl-2-nitrothiophenol sodium salt, 4-chlorosulfonyl-2-aminothiophenol sodium salt, 4-chlorosulfonyl-2-hydroxythiophenol sodium salt, 4-chlorosulfonyl-2-phenylthiothiophenol sodium salt, 4-sulfino-2-nitrothiophenol sodium salt, 4-sulfino-2-aminothiophenol sodium salt, 4-sulfino-2-hydroxythiophenol sodium salt, 4-sulfino-2-phenylthiothiophenol sodium salt, 4-methylsulfinyl-2-nitrothiophenol sodium salt, 4-methylsulfinyl-2-aminothiophenol sodium salt, 4-methylsulfinyl-2-hydroxythiophenol sodium salt, 4-methylsulfinyl-2-phenylthiothiophenol sodium salt, 4-carbamoyl-2-nitrothiophenol sodium salt, 4-carbamoyl-2-aminothiophenol sodium salt, 4-carbamoyl-2-hydroxythiophenol sodium salt, 4-carbamoyl-2-phenylthiothiophenol sodium salt, 4-trichloromethyl-2-nitrothiophenol sodium salt, 4-trichloromethyl-2-aminothiophenol sodium salt, 4-trichloromethyl-2-hydroxythiophenol sodium salt, 4-trichloromethyl-2-phenylthiothiophenol sodium salt, 4-cyano-2-nitrothiophenol sodium salt, 4-cyano-2-aminothiophenol sodium salt, 4-cyano-2-hydroxythiophenol sodium salt, 4-cyano-2-phenylthiothiophenol sodium salt, 4-methoxy-2-nitrothiophenol sodium salt, 4-methoxy-2-aminothiophenol sodium salt, 4-methoxy-2-hydroxythiophenol sodium salt, and 4-methoxy-2-phenylthiothiophenol sodium salt.

Still another example of the organic sulfur compound represented by the chemical formula (3) is a compound substituted with two or more types of substituents. Specific examples of the compound include 4-acetyl-2-chlorothiophenol sodium salt, 4-acetyl-2-methylthiophenol sodium salt, 4-acetyl-2-carboxythiophenol sodium salt, 4-acetyl-2-methoxycarbonylthiophenol sodium salt, 4-acetyl-2-formylthiophenol sodium salt, 4-acetyl-2-chlorocarbonylthiophenol sodium salt, 4-acetyl-2-sulfothiophenol sodium salt, 4-acetyl-2-methoxysulfonylthiophenol sodium salt, 4-acetyl-2-chlorosulfonylthiophenol sodium salt, 4-acetyl-2-sulfinothiophenol sodium salt, 4-acetyl-2-methylsulfinylthiophenol sodium salt, 4-acetyl-2-carbamoylthiophenol sodium salt, 4-acetyl-2-trichloromethylthiophenol sodium salt, 4-acetyl-2-cyanothiophenol sodium salt, and 4-acetyl-2-methoxythiophenol sodium salt. Examples of the monovalent metal represented by M1 in the chemical formula (3) include sodium, lithium, potassium, copper (I), and silver (I) .

Examples of the organic sulfur compound represented by the chemical formula (4) include thiophenol zinc salt; thiophenol zinc salts substituted with halogen groups, such as 4-fluorothiophenol zinc salt, 2,5-difluorothiophenol zinc salt, 2,4,5-trifluorothiophenol zinc salt, 2,4,5,6-tetrafluorothiophenol zinc salt, pentafluorothiophenol zinc salt, 4-chlorothiophenol zinc salt, 2,5-dichlorothiophenol zinc salt, 2,4,5-trichlorothiophenol zinc salt, 2,4,5,6-tetrachlorothiophenol zinc salt, pentachlorothiophenol zinc salt, 4-bromothiophenol zinc salt, 2,5-dibromothiophenolzinc salt,2,4,5-tribromothiophenol zinc salt, 2,4,5,6-tetrabromothiophenol zinc salt, pentabromothiophenol zinc salt, 4-iodothiophenol zinc salt, 2,5-diiodothiophenol zinc salt, 2,4,5-triiodothiophenol zinc salt, 2,4,5,6-tetraiodothiophenol zinc salt, and pentaiodothiophenol zinc salt; thiophenol zinc salts substituted with alkyl groups, such as 4-methylthiophenol zinc salt, 2,4,5-trimethylthiophenol zinc salt, pentamethylthiophenol zinc salt, 4-t-butylthiophenol zinc salt, 2,4,5-tri-t-butylthiophenol zinc salt, and penta-t-butylthiophenol zinc salt; thiophenol zinc salts substituted with carboxyl groups, such as 4-carboxythiophenol zinc salt, 2,4,6-tricarboxythiophenol zinc salt, and pentacarboxythiophenol zinc salt; thiophenol zinc salts substituted with alkoxycarbonyl groups, such as 4-methoxycarbonylthiophenol zinc salt, 2,4,6-trimethoxycarbonylthiophenol zinc salt, and pentamethoxycarbonylthiophenol zinc salt; thiophenol zinc salts substituted with formyl groups, such as 4-formylthiophenol zinc salt, 2,4,6-triformylthiophenol zinc salt, and pentaformylthiophenol zinc salt; thiophenol zinc salts substituted with acyl groups, such as 4-acetylthiophenol zinc salt, 2,4,6-triacetylthiophenol zinc salt, and pentaacetylthiophenol zinc salt; thiophenol zinc salts substituted with carbonyl halide groups, such as 4-chlorocarbonylthiophenol zinc salt, 2,4,6-tri(chlorocarbonyl)thiophenol zinc salt, and penta(chlorocarbonyl)thiophenol zinc salt; thiophenol zinc salts substituted with sulfo groups, such as 4-sulfothiophenol zinc salt, 2,4,6-trisulfothiophenol zinc salt, and pentasulfothiophenol zinc salt; thiophenol zinc salts substituted with alkoxysulfonyl groups, such as 4-methoxysulfonylthiophenol zinc salt, 2,4,6-trimethoxysulfonylthiophenol zinc salt, and pentamethoxysulfonylthiophenol zinc salt; thiophenol zinc salts substituted with sulfonyl halide groups, such as 4-chlorosulfonylthiophenol zinc salt, 2,4,6-tri(chlorosulfonyl)thiophenol zinc salt, and penta(chlorosulfonyl)thiophenol zinc salt; thiophenol zinc salts substituted with sulfino groups, such as 4-sulfinothiophenolzincsalt, 2,4,6-trisulfinothiophenolzinc salt, and pentasulfinothiophenol zinc salt; thiophenol zinc salts substituted with alkylsulfinyl groups, such as 4-methylsulfinylthiophenol zinc salt, 2,4,6-tri(methylsulfinyl)thiophenol zinc salt, and penta(methylsulfinyl)thiophenol zinc salt; thiophenol zinc salts substituted with carbamoyl groups, such as 4-carbamoylthiophenol zinc salt, 2,4,6-tricarbamoylthiophenol zinc salt, and pentacarbamoylthiophenol zinc salt; thiophenol zinc salts substituted with alkyl halide groups, such as 4-trichloromethylthiophenol zinc salt, 2,4,6-tri(trichloromethyl)thiophenol zinc salt, and penta(trichloromethyl)thiophenol zinc salt; thiophenol zinc salts substituted with cyano groups, such as 4-cyanothiophenol zinc salt, 2,4,6-tricyanothiophenol zinc salt, and pentacyanothiophenol zinc salt; and thiophenol zinc salts substituted with alkoxy groups, such as 4-methoxythiophenol zinc salt, 2,4,6-trimethoxythiophenol zinc salt, and pentamethoxythiophenol zinc salt. Each of these thiophenol zinc salts is substituted with one type of substituent.

Another example of the organic sulfur compound represented by the chemical formula (4) is a compound substituted with at least one type of the above substituents and another substituent. Examples of the other substituent include a nitro group (-NO₂), an amino group (-NH₂), a hydroxyl group (-OH), and a phenylthio group (-SPh). Specific examples of the compound include 4-chloro-2-nitrothiophenol zinc salt, 4-chloro-2-aminothiophenol zinc salt, 4-chloro-2-hydroxythiophenol zinc salt, 4-chloro-2-phenylthiothiophenol zinc salt, 4-methyl-2-nitrothiophenol zinc salt, 4-methyl-2-aminothiophenol zinc salt, 4-methyl-2-hydroxythiophenol zinc salt, 4-methyl-2-phenylthiothiophenol zinc salt, 4-carboxy-2-nitrothiophenol zinc salt, 4-carboxy-2-aminothiophenol zinc salt, 4-carboxy-2-hydroxythiophenol zinc salt, 4-carboxy-2-phenylthiothiophenol zinc salt, 4-methoxycarbonyl-2-nitrothiophenol zinc salt, 4-methoxycarbonyl-2-aminothiophenol zinc salt, 4-methoxycarbonyl-2-hydroxythiophenol zinc salt, 4-methoxycarbonyl-2-phenylthiothiophenol zinc salt, 4-formyl-2-nitrothiophenol zinc salt, 4-formyl-2-aminothiophenol zinc salt, 4-formyl-2-hydroxythiophenol zinc salt, 4-formyl-2-phenylthiothiophenol zinc salt, 4-acetyl-2-nitrothiophenol zinc salt, 4-acetyl-2-aminothiophenol zinc salt, 4-acetyl-2-hydroxythiophenol zinc salt, 4-acetyl-2-phenylthiothiophenol zinc salt, 4-chlorocarbonyl-2-nitrothiophenol zinc salt, 4-chlorocarbonyl-2-aminothiophenol zinc salt, 4-chlorocarbonyl-2-hydroxythiophenol zinc salt, 4-chlorocarbonyl-2-phenylthiothiophenol zinc salt, 4-sulfo-2-nitrothiophenol zinc salt, 4-sulfo-2-aminothiophenol zinc salt, 4-sulfo-2-hydroxythiophenol zinc salt, 4-sulfo-2-phenylthiothiophenol zinc salt, 4-methoxysulfonyl-2-nitrothiophenol zinc salt, 4-methoxysulfonyl-2-aminothiophenol zinc salt, 4-methoxysulfonyl-2-hydroxythiophenol zinc salt, 4-methoxysulfonyl-2-phenylthiothiophenol zinc salt, 4-chlorosulfonyl-2-nitrothiophenol zinc salt, 4-chlorosulfonyl-2-aminothiophenol zinc salt, 4-chlorosulfonyl-2-hydroxythiophenol zinc salt, 4-chlorosulfonyl-2-phenylthiothiophenol zinc salt, 4-sulfino-2-nitrothiophenol zinc salt, 4-sulfino-2-aminothiophenol zinc salt, 4-sulfino-2-hydroxythiophenol zinc salt, 4-sulfino-2-phenylthiothiophenol zinc salt, 4-methylsulfinyl-2-nitrothiophenol zinc salt, 4-methylsulfinyl-2-aminothiophenol zinc salt, 4-methylsulfinyl-2-hydroxythiophenol zinc salt, 4-methylsulfinyl-2-phenylthiothiophenol zinc salt, 4-carbamoyl-2-nitrothiophenol zinc salt, 4-carbamoyl-2-aminothiophenol zinc salt, 4-carbamoyl-2-hydroxythiophenol zinc salt, 4-carbamoyl-2-phenylthiothiophenol zinc salt, 4-trichloromethyl-2-nitrothiophenol zinc salt, 4-trichloromethyl-2-aminothiophenol zinc salt, 4-trichloromethyl-2-hydroxythiophenol zinc salt, 4-trichloromethyl-2-phenylthiothiophenol zinc salt, 4-cyano-2-nitrothiophenol zinc salt, 4-cyano-2-aminothiophenol zinc salt, 4-cyano-2-hydroxythiophenol zinc salt, 4-cyano-2-phenylthiothiophenol zinc salt, 4-methoxy-2-nitrothiophenol zinc salt, 4-methoxy-2-aminothiophenol zinc salt, 4-methoxy-2-hydroxythiophenol zinc salt, and 4-methoxy-2-phenylthiothiophenol zinc salt.

Still another example of the organic sulfur compound represented by the chemical formula (4) is a compound substituted with two or more types of substituents. Specific examples of the compound include 4-acetyl-2-chlorothiophenol zinc salt, 4-acetyl-2-methylthiophenol zinc salt, 4-acetyl-2-carboxythiophenol zinc salt, 4-acetyl-2-methoxycarbonylthiophenol zinc salt, 4-acetyl-2-formylthiophenol zinc salt, 4-acetyl-2-chlorocarbonylthiophenol zinc salt, 4-acetyl-2-sulfothiophenol zinc salt, 4-acetyl-2-methoxysulfonylthiophenol zinc salt, 4-acetyl-2-chlorosulfonylthiophenol zinc salt, 4-acetyl-2-sulfinothiophenol zinc salt, 4-acetyl-2-methylsulfinylthiophenol zinc salt, 4-acetyl-2-carbamoylthiophenol zinc salt, 4-acetyl-2-trichloromethylthiophenol zinc salt, 4-acetyl-2-cyanothiophenol zinc salt, and 4-acetyl-2-methoxythiophenol zinc salt. Examples of the bivalent metal represented by M2 in the chemical formula (4) include zinc, magnesium, calcium, strontium, barium, titanium (II), manganese (II), iron (II), cobalt (II), nickel (II), zirconium (II), and tin (II).

Examples of thionaphthols include 2-thionaphthol, 1-thionaphthol, 2-chloro-1-thionaphthol, 2-bromo-1-thionaphthol, 2-fluoro-1-thionaphthol, 2-cyano-1-thionaphthol, 2-acetyl-1-thionaphthol, 1-chloro-2-thionaphthol, 1-bromo-2-thionaphthol, 1-fluoro-2-thionaphthol, 1-cyano-2-thionaphthol, 1-acetyl-2-thionaphthol, and metal salts thereof. 1-thionaphthol, 2-thionaphthol, and zinc salts thereof are preferred.

Examples of sulfenamide type organic sulfur compounds include N-cyclohexyl-2-benzothiazole sulfenamide, N-oxydiethylene-2-benzothiazole sulfenamide, and N-t-butyl-2-benzothiazole sulfenamide. Examples of thiuram type organic sulfur compounds include tetramethylthiuram monosulfide, tetramethylthiuram disulfide, tetraethylthiuram disulfide, tetrabutylthiuram disulfide, and dipentamethylenethiuram tetrasulfide. Examples of dithiocarbamates include zinc dimethyldithiocarbamate, zinc diethyldithiocarbamate, zinc dibutyldithiocarbamate, zinc ethylphenyldithiocarbamate, sodium dimethyldithiocarbamate, sodium diethyldithiocarbamate, copper (II) dimethyldithiocarbamate, iron (III) dimethyldithiocarbamate, selenium diethyldithiocarbamate, and tellurium diethyldithiocarbamate. Examples of thiazole type organic sulfur compounds include 2-mercaptobenzothiazole (MBT); dibenzothiazyl disulfide (MBTS); a sodium salt, a zinc salt, a copper salt, and a cyclohexylamine salt of 2-mercaptobenzothiazole; 2-(2,4-dinitrophenyl)mercaptobenzothiazole; and 2-(2,6-diethyl-4-morpholinothio)benzothiazole.

Particularly preferable organic sulfur compounds (e) from the standpoint that an outer-hard/inner-soft structure is easily obtained are 2-thionaphthol, bis(pentabromophenyl)disulfide, and 2,6-dichlorothiophenol.

In light of an outer-hard/inner-soft structure of the core 4, the amount of the organic sulfur compound (f) is preferably equal to or greater than 0.05 parts by weight, more preferably equal to or greater than 0.1 parts by weight, and particularly preferably equal to or greater than 0.2 parts by weight, per 100 parts by weight of the base rubber. In light of resilience performance, the amount is preferably equal to or less than 5 parts by weight, more preferably equal to or less than 3 parts by weight, and particularly preferably equal to or less than 1 parts by weight, per 100 parts by weight of the base rubber.

For the purpose of adjusting specific gravity and the like, a filler may be included in the core 4. Examples of suitable fillers include zinc oxide, barium sulfate, calcium carbonate, and magnesium carbonate . The amount of the filler is determined as appropriate so that the intended specific gravity of the core 4 is accomplished. A particularly preferable filler is zinc oxide. Zinc oxide serves not only as a specific gravity adjuster but also as a crosslinking activator.

According to need, an anti-aging agent, a coloring agent, a plasticizer, a dispersant, sulfur, a vulcanization accelerator, and the like are added to the rubber composition of the core 4. Crosslinked rubber powder or synthetic resin powder may also be dispersed in the rubber composition.

During heating and forming of the core 4, the heat of the crosslinking reaction of the base rubber remains near the central point of the core 4. Thus, during heating and forming of the core 4, the temperature at the central portion is high. The temperature gradually decreases from the central point toward the surface. The acid and/or the salt (d) reacts with a metal salt of the co-crosslinking agent (b) to break metal crosslinks. This reaction is accelerated in a region where the temperature is high. In other words, breaking of the metal crosslinks is likely to occur in the central portion of the core 4 where the temperature is high, and is unlikely to occur near the surface of the core 4. As a result, the crosslinking density of the core 4 increases from its central point toward its surface. In the core 4, the hardness linearly increases from its central point toward its surface. Furthermore, since the rubber composition includes the organic sulfur compound (f) together with the acid and/or the salt (d), the gradient of the hardness distribution can be controlled, and the degree of the outer-hard/inner-soft structure of the core 4 can be increased.

FIG. 2 is a line graph showing a hardness distribution of the core 4 of the golf ball 2 in FIG. 1 according to the present invention. The horizontal axis of the graph indicates the ratio (%) of a distance from the central point of the core 4 to the radius of the core 4. The vertical axis of the graph indicates a JIS-C hardness. Nine measuring points obtained by dividing a region from the central point of the core 4 to the surface of the core 4 at intervals of 12.5% of the radius of the core 4 are plotted in the graph. The ratio of the distance from the central point of the core 4 to each of these measuring points to the radius of the core 4 is as follows.
First point: 0.0% (central point)
Second point: 12.5%
Third point: 25.0%
Fourth point: 37.5%
Fifth point: 50.0%
Sixth point: 62.5%
Seventh point: 75.0%
Eighth point: 87.5%
Ninth point: 100.0% (surface)

Hardnesses at the first to eighth points are measured by pressing a JIS-C type hardness scale against a cut plane of the core 4 that has been cut into two halves. A hardness at the ninth point is measured by pressing the JIS-C type hardness scale against the surface of the spherical core 4. For the measurement, an automated rubber hardness measurement machine (trade name "P1", manufactured by Kobunshi Keiki Co., Ltd.), to which this hardness scale is mounted, is used.

FIG. 2 also shows a linear approximation curve obtained by a least-square method on the basis of the distances and the hardnesses of the nine measuring points. In FIG. 2, the broken line does not greatly deviate from the linear approximation curve. In other words, the broken line has a shape close to the linear approximation curve. That is, in the core 4 according to the present invention, the hardness linearly increases from its central point toward its surface. When the golf ball 2 that includes the core 4 is hit with a driver, the energy loss is low. The core 4 has excellent resilience performance. When the golf ball 2 is hit with a driver, the flight distance is large. In the core 4, the hardness continuously increases from its central point toward its surface. In the core 4, there is no discontinuous point caused by a multilayer structure. When the golf ball 2 that includes the core 4 deforms by being hit, no local load is applied thereto. The golf ball 2 has excellent durability.

In the core 4, R² of the linear approximation curve obtained by the least-square method is equal to or greater than 0.95. R² is an index indicating the linearity of the broken line. For the core 4 for which R² is equal to or greater than 0.95, the shape of the broken line of the hardness distribution is close to a straight line. The core 4 for which R² is equal to or greater than 0.95 has excellent resilience performance. In this respect, R² is more preferably equal to or greater than 0.97 and particularly preferably equal to or greater than 0.99. R² is calculated by squaring a correlation coefficient R. The correlation coefficient R is calculated by dividing the covariance of the distance (%) from the central point and the hardness (JIS-C) by the standard deviation of the distance (%) from the central point and the standard deviation of the hardness (JIS-C) .

In the present invention, a JIS-C hardness at a measuring point whose ratio of the distance from the central point of the core 4 to the radius of the core 4 is x% is represented by H(x). The hardness at the central point of the core 4 is represented by H(0.0). The surface hardness of the core 4 is represented by Hs. The difference (Hs-H(0.0)) between the surface hardness Hs and the central hardness H(0.0) is equal to or greater than 15. The difference is great. In other words, the core 4 has an outer-hard/inner-soft structure. When the core 4 is hit with a driver, the recoil (torsional return) is great, and thus spin is suppressed. The core 4 contributes to the flight performance of the golf ball 2. In light of flight performance, the difference (Hs-H(0.0)) is more preferably equal to or greater than 25 and particularly preferably equal to or greater than 30. From the standpoint that the core 4 can easily be formed, the difference (Hs-H(0.0)) is preferably equal to or less than 50.

The hardness H(0.0) at the central point of the core 4 is preferably equal to or greater than 40 but equal to or less than 70. The golf ball 2 that includes the core 4 having a hardness H(0.0) of 40 or greater has excellent resilience performance. The hardness H(0.0) is more preferably equal to or greater than 45 and particularly preferably equal to or greater than 50. In the core 4 having a hardness H(0.0) of 70 or less, an outer-hard/inner-soft structure can be achieved. In the golf ball 2 that includes the core 4, spin can be suppressed. The hardness H(0.0) is more preferably equal to or less than 68 and particularly preferably equal to or less than 65.

The hardness Hs at the surface of the core 4 is preferably equal to or greater than 78 but equal to or less than 96. In the core 4 having a hardness Hs of 78 or greater, an outer-hard/inner-soft structure can be achieved. In the golf ball 2 that includes the core 4, spin can be suppressed. The hardness Hs is more preferably equal to or greater than 80 and particularly preferably equal to or greater than 82. The golf ball 2 that includes the core 4 having a hardness Hs of 96 or less has excellent durability. The hardness Hs is more preferably equal to or less than 94 and particularly preferably equal to or less than 92.

The core 4 has a diameter of 36.0 mm or greater. The core 4 having a diameter of 36.0 mm or greater can achieve excellent resilience performance of the golf ball 2. The core 4 having a diameter of 36.0 mm or greater can achieve an outer-hard/inner-soft structure of the golf ball 2. In this respect, the diameter is preferably equal to or greater than 37.0 mm and particularly preferably equal to or greater than 38.0 mm. Furthermore, the diameter of the core 4 is preferably equal to or less than 40.1 mm. In the golf ball 2 that includes the core 4 having a diameter of 40.1 mm or less, the inner mid layer 6, the outer mid layer 8, and the cover 12 can have sufficient thicknesses. The golf ball 2 that includes the inner mid layer 6, the outer mid layer 8, and the cover 12 which have large thicknesses has excellent durability. In this respect; the diameter is particularly preferably equal to or less than 38.8 mm.

In light of feel at impact, the core 4 has an amount of compressive deformation Dc of preferably 3.0 mm or greater and particularly preferably 3.2 mm or greater. In light of resilience performance, the amount of compressive deformation Dc is preferably equal to or less than 3.8 mm and particularly preferably equal to or less than 3.5 mm.

For the inner mid layer 6, a resin composition is suitably used. Examples of the base resin of the resin composition include ionomer resins, polystyrenes, polyesters, polyamides, and polyolefins.

Particularly preferable base resins are ionomer resins. The golf ball 2 that includes the inner mid layer 6 including an ionomer resin has excellent resilience performance. An ionomer resin and another resin may be used in combination for the inner mid layer 6. In this case, the principal component of the base resin is preferably the ionomer resin. Specifically, the proportion of the ionomer resin to the entire base resin is preferably equal to or greater than 80% by weight and more preferably equal to or greater than 90% by weight.

Examples of preferable ionomer resins include binary copolymers formed with an α-olefin and an α,β-unsaturated carboxylic acid having 3 to 8 carbon atoms . A preferable binary copolymer includes 80% by weight or greater but 90% by weight or less of an α-olefin, and 10% by weight or greater but 20% by weight or less of an α,β-unsaturated carboxylic acid. The binary copolymer has excellent resilience performance. Examples of other preferable ionomer resins include ternary copolymers formed with: an α-olefin; an α,β-unsaturated carboxylic acid having 3 to 8 carbon atoms; and an α,β-unsaturated carboxylate ester having 2 to 22 carbon atoms. A preferable ternary copolymer includes 70% by weight or greater but 85% by weight or less of an α-olefin, 5% by weight or greater but 30% by weight or less of an α,β-unsaturated carboxylic acid, and 1% by weight or greater but 25% by weight or less of an α,β-unsaturated carboxylate ester. The ternary copolymer has excellent resilience performance. For the binary copolymers and the ternary copolymers, preferable α-olefins are ethylene and propylene, while preferable α,β-unsaturated carboxylic acids are acrylic acid and methacrylic acid. A particularly preferable ionomer resin is a copolymer formed with ethylene and acrylic acid or methacrylic acid.

In the binary copolymers and the ternary copolymers, some of the carboxyl groups are neutralized with metal ions. Examples of metal ions for use in neutralization include sodium ion, potassium ion, lithium ion, zinc ion, calcium ion, magnesium ion, aluminum ion, and neodymium ion. The neutralization may be carried out with two or more types of metal ions. Particularly suitable metal ions in light of resilience performance and durability of the golf ball 2 are sodium ion, zinc ion, lithium ion, and magnesium ion.

Specific examples of ionomer resins include trade names "Himilan1555", "Himilan1557", "Himilan1605", "Himilan1706", "Himilan 1707", "Himilan 1856", "Himilan 1855", "Himilan AM7311", "Himilan AM7315", "Himilan AM7317", "Himilan AM7318", "Himilan AM7329", "Himilan MK7320", and "Himilan MK7329", manufactured by Du Pont-MITSUI POLYCHEMICALS Co., Ltd.; trade names "Surlyn 6120", "Surlyn 6910", "Surlyn 7930", "Surlyn 7940", "Surlyn 8140", "Surlyn 8150", "Surlyn 8940", "Surlyn 8945", "Surlyn 9120", "Surlyn 9150", "Surlyn 9910", "Surlyn 9945", "Surlyn AD8546", "HPF1000", and "HPF2000", manufactured by E.I. du Pont de Nemours and Company; and trade names "IOTEK 7010", "IOTEK 7030", "IOTEK 7510", "IOTEK 7520", "IOTEK 8000", and "IOTEK 8030", manufactured by ExxonMobil Chemical Company.

Two or more ionomer resins may be used in combination for the inner mid layer 6. An ionomer resin neutralized with a monovalent metal ion, and an ionomer resin neutralized with a bivalent metal ion may be used in combination.

In the inner mid layer 6, a highly elastic resin may be included. Specific examples of the highly elastic resin include polyamides.

According to need, a coloring agent such as titanium dioxide, a filler such as barium sulfate, a dispersant, an antioxidant, an ultraviolet absorber, a light stabilizer, a fluorescent material, a fluorescent brightener, and the like are included in the resin composition of the inner mid layer 6 in an adequate amount.

From the standpoint that an outer-hard/inner-soft structure can be achieved in the sphere consisting of the core 4 and the inner mid layer 6, the inner mid layer 6 has a Shore D hardness Hm1 of preferably 55 or greater and more preferably 60 or greater. In the golf ball 2 that includes the inner mid layer 6 having a hardness Hm1 in this range, a spin rate is sufficiently suppressed upon a shot with a driver. The flight distance of the golf ball 2 is large. In light of controllability of the golf ball 2, the hardness Hm1 is preferably equal to or less than 70 and particularly preferably equal to or less than 68. When the golf ball 2 is hit with a short iron, the spin rate is high.

The Shore D hardness Hm1 of the inner mid layer 6 is measured according to the standards of "ASTM-D 2240-68" with a Shore D type hardness scale mounted to an automated rubber hardness measurement machine (trade name "P1", manufactured by Kobunshi Keiki Co., Ltd.). For the measurement, a slab that is formed by hot press and that has a thickness of about 2 mm is used. A slab kept at 23°C for two weeks is used for the measurement. At the measurement, three slabs are stacked. A slab formed from the same resin composition as the resin composition of the inner mid layer 6 is used.

The inner mid layer 6 preferably has a thickness T1 of 0.5 mm or greater but 1.6 mm or less. In light of durability, the thickness T1 is more preferably equal to or greater than 0.7 mm. In light of resilience performance, the thickness T1 is more preferably equal to or less than 1.2 mm.

For the outer mid layer 8, a resin composition is suitably used. Examples of the base resin of the resin composition include ionomer resins, polystyrenes, polyesters, polyamides, and polyolefins.

Particularly preferable base resins are ionomer resins. The ionomer resins described above for the inner mid layer 6 can also be used for the outer mid layer 8. The golf ball 2 that includes the outer mid layer 8 including an ionomer resin has excellent resilience performance. An ionomer resin and another resin may be used in combination for the outer mid layer 8. In this case, the principal component of the base resin is preferably the ionomer resin. Specifically, the proportion of the ionomer resin to the entire base resin is preferably equal to or greater than 45% by weight and more preferably equal to or greater than 60% by weight.

A preferable resin that can be used in combination with an ionomer resin is a styrene block-containing thermoplastic elastomer. The styrene block-containing thermoplastic elastomer has excellent compatibility with ionomer resins. A resin composition including the styrene block-containing thermoplastic elastomer has excellent fluidity.

The styrene block-containing thermoplastic elastomer includes a polystyrene block as a hard segment, and a soft segment. A typical soft segment is a diene block. Examples of compounds for the diene block include butadiene, isoprene, 1,3-pentadiene, and 2,3-dimethyl-1,3-butadiene. Butadiene and isoprene are preferred. Two or more compounds may be used in combination.

Examples of styrene block-containing thermoplastic elastomers include styrene-butadiene-styrene block copolymers (SBS), styrene-isoprene-styrene block copolymers (SIS), styrene-isoprene-butadiene-styrene block copolymers (SIBS), hydrogenated SBS, hydrogenated SIS, and hydrogenated SIBS. Examples of hydrogenated SBS include styrene-ethylene-butylene-styrene block copolymers (SEBS). Examples of hydrogenated SIS include styrene-ethylene-propylene-styrene block copolymers (SEPS). Examples of hydrogenated SIBS include styrene-ethylene-ethylene-propylene-styrene block copolymers (SEEPS).

In light of resilience performance of the golf ball 2, the content of the styrene component in the styrene block-containing thermoplastic elastomer is preferably equal to or greater than 10% by weight, more preferably equal to or greater than 12% by weight, and particularly preferably equal to or greater than 15% by weight. In light of feel at impact of the golf ball 2, the content is preferably equal to or less than 70% by weight, more preferably equal to or less than 65% by weight, and particularly preferably equal to or less than 60% by weight.

In the present invention, styrene block-containing thermoplastic elastomers include a polymer alloy of an olefin and one or more members selected from the group consisting of SBS, SIS, SIBS, and a hydrogenated product thereof. The olefin component in the polymer alloy is presumed to contribute to improvement of compatibility with ionomer resins. Use of this polymer alloy improves the resilience performance of the golf ball 2. An olefin having 2 to 10 carbon atoms is preferably used. Examples of suitable olefins include ethylene, propylene, butene, and pentene. Ethylene and propylene are particularly preferred.

Specific examples of polymer alloys include trade names "RabalonT3221C", "RabalonT3339C", "RabalonSJ4400N", "Rabalon SJ5400N", "Rabalon SJ6400N", "Rabalon SJ7400N", "Rabalon SJ8400N", "Rabalon SJ9400N", and "Rabalon SR04", manufactured by Mitsubishi Chemical Corporation. Other specific examples of styrene block-containing thermoplastic elastomers include trade name "Epofriend A1010" manufactured by Daicel Chemical Industries, Ltd., and trade name "Septon HG-252" manufactured by Kuraray Co., Ltd.

According to need, a coloring agent such as titanium dioxide, a filler such as barium sulfate, a dispersant, an antioxidant, an ultraviolet absorber, a light stabilizer, a fluorescent material, a fluorescent brightener, and the like are included in the resin composition of the outer mid layer 8 in an adequate amount.

In light of a spin suppression effect upon a shot with a driver, the outer mid layer 8 has a Shore D hardness Hm2 of preferably 25 or greater and more preferably 30 or greater. The flight distance of the golf ball 2 is large. In light of controllability of the golf ball 2, the hardness Hm2 is preferably equal to or less than 60 and particularly preferably equal to or less than 54. When the golf ball 2 is hit with a short iron, the spin rate is high. The hardness Hm2 is measured by the same measurement method as that for the hardness Hm1.

In light of durability and feel at impact, the hardness Hm1 of the inner mid layer 6 is preferably greater than the hardness Hm2 of the outer mid layer 8. When the golf ball 2 in which the hardness Hm1 is greater than the hardness Hm2 is hit with a driver, the shock provided to the golf ball 2 by the driver is alleviated. The golf ball 2 has excellent durability. The golf ball 2 has soft feel at impact.

The difference (Hm1-Hm2) between the hardness Hm1 of the inner mid layer 6 and the hardness Hm2 of the outer mid layer 8 is preferably equal to or greater than 8 and particularly preferably equal to or greater than 14. In light of resilience performance, the difference (Hm1-Hm2) is preferably equal to or less than 35. When the golf ball 2 that includes the outer mid layer 8 having a hardness Hm2 in this range is hit with a driver, the spin rate is low. The flight distance of the golf ball 2 is large. When the golf ball 2 is hit with a short iron, the spin rate is high.

The outer mid layer 8 preferably has a thickness T2 of 0.5 mm or greater. In the golf ball 2 that includes the outer mid layer 8 having a thickness T2 of 0.5 mm or greater, the shock by a hit is alleviated. Thus, the golf ball 2 has excellent durability. In this respect, the thickness T2 is more preferably equal to or greater than 0.7 mm. The thickness T2 is preferably equal to or less than 1.6 mm. The golf ball 2 that includes the outer mid layer 8 having a thickness T2 of 1.6 mm or less includes a relatively large core 4. The golf ball 2 exerts sufficient resilience performance. In this respect, the thickness T2 is particularly preferably equal to or less than 1.2 mm.

The sum (T1+T2) of the thickness T1 and the thickness T2 is preferably equal to or greater than 1.0 mm. In the golf ball 2, the shock by a hit is alleviated. Thus, the golf ball 2 has excellent durability. In this respect, the sum (T1+T2) is more preferably equal to or greater than 1.3 mm. The sum (T1+T2) is preferably equal to or less than 3.0 mm. The golf ball 2 includes a relatively large core 4. The golf ball 2 exerts sufficient resilience performance. In this respect, the sum (T1+T2) is more preferably equal to or less than 2.0 mm.

For forming the outer mid layer 8, known methods such as injection molding, compression molding, and the like can be used.

For the cover 12, a resin composition is suitably used. A preferable base resin of the resin composition is a urethane resin or a urea resin. The principal component of the urethane resin is a polyurethane. The polyurethane is flexible. When the golf ball 2 that includes the cover 12 formed from the resin composition that includes the polyurethane is hit with a short iron, the spin rate is high. The cover 12 formed from this resin composition contributes to controllability upon a shot with a short iron. The polyurethane also contributes to the scuff resistance of the cover 12. Furthermore, the polyurethane can also contribute to excellent feel at impact when the golf ball 2 is hit with a putter or a short iron.

In light of ease of forming the cover 12, a preferable base resin is a thermoplastic polyurethane elastomer. The thermoplastic polyurethane elastomer includes a polyurethane component as a hard segment, and a polyester component or a polyether component as a soft segment. Examples of isocyanates for the polyurethane component include alicyclic diisocyanates, aromatic diisocyanates, and aliphatic diisocyanates. Two or more diisocyanates may be used in combination.

Examples of alicyclic diisocyanates include 4,4'-dicyclohexylmethane diisocyanate (H₁₂MDI), 1,3-bis(isocyanatomethyl)cyclohexane (H₆XDI), isophorone diisocyanate (IPDI), and trans-1,4-cyclohexane diisocyanate (CHDI) . In light of versatility and processability, H₁₂MDI is preferred.

Examples of aromatic diisocyanates include 4,4'-diphenylmethane diisocyanate (MDI) and toluene diisocyanate (TDI). Examples of aliphatic diisocyanates include hexamethylene diisocyanate (HDI).

Particularly, alicyclic diisocyanates are preferred. Since an alicyclic diisocyanate does not have any double bond in the main chain, the alicyclic diisocyanate suppresses yellowing of the cover 12. In addition, since an alicyclic diisocyanate has excellent strength, the alicyclic diisocyanate suppresses a scuff on the cover 12.

Specific examples of thermoplastic polyurethane elastomers include trade names "Elastollan NY80A", "Elastollan NY82A", "Elastollan NY84A", "Elastollan NY85A", "Elastollan NY88A", "Elastollan NY90A", "Elastollan NY97A", "Elastollan NY585", "Elastollan XKP016N", "Elastollan 1195ATR", "Elastollan ET890A", and "Elastollan ET88050", manufactured by BASF Japan Ltd.; and trade names "RESAMINE P4585LS" and "RESAMINE PS62490", manufactured by Dainichiseika Color & Chemicals Mfg. Co., Ltd. From the standpoint that a low hardness of the cover 12 can be achieved, "Elastollan NY80A", "Elastollan NY82A", "Elastollan NY84A", "ElastollanNY85A", "Elastollan NY90A", and "Elastollan NY97A" are particularly preferred.

A thermoplastic polyurethane elastomer and another resin may be used in combination. Examples of the resin that can be used in combination include thermoplastic polyester elastomers, thermoplastic polyamide elastomers, thermoplastic polyolefin elastomers, styreneblock-containing thermoplastic elastomers, and ionomer resins. When a thermoplastic polyurethane elastomer and another resin are used in combination, the thermoplastic polyurethane elastomer is included as the principal component of the base polymer, in light of spin performance and scuff resistance. The proportion of the thermoplastic polyurethane elastomer to the entire base polymer is preferably equal to or greater than 50% by weight, more preferably equal to or greater than 70% by weight, and particularly preferably equal to or greater than 85% by weight.

According to need, a coloring agent such as titanium dioxide, a filler such as barium sulfate, a dispersant, an antioxidant, an ultraviolet absorber, a light stabilizer, a fluorescent material, a fluorescent brightener, and the like are included in the cover 12 in an adequate amount.

The cover 12 preferably has a Shore D hardness Hc of 48 or less. The golf ball 2 that includes the cover 12 having a hardness Hc of 48 or less has excellent controllability. In this respect, the hardness Hc is more preferably equal to or less than 40 and particularly preferably equal to or less than 32. In light of flight distance upon a shot with a driver, the hardness Hc is preferably equal to or greater than 10, more preferably equal to or greater than 15, and particularly preferably equal to or greater than 20. The hardness Hc is measured by the same measurement method as that for the hardness Hm1 and the hardness Hm2.

The hardness Hc of the cover 12 is less than the hardness Hm1 of the inner mid layer 6. When the golf ball 2 is hit with a driver, the sphere consisting of the core 4 and the inner mid layer 6 becomes significantly distorted since the head speed is high. Since this sphere has an outer-hard/inner-soft structure, the spin rate is suppressed. The hardness of the core 4 linearly changes. Thus, the golf ball 2 is launched at a high speed due to deformation and restoration of the core 4. The suppression of the spin rate and the high launch speed achieve a large flight distance. When the golf ball 2 is hit with a short iron, this sphere becomes less distorted since the head speed is low. When the golf ball 2 is hit with a short iron, the behavior of the golf ball 2 mainly depends on the cover 12. Since the cover 12 is flexible, a slip between the golf ball 2 and a clubface is suppressed. Due to the suppression of the slip, a high spin rate is obtained. The high spin rate achieves excellent controllability. In the golf ball 2, both desired flight performance upon a shot with a driver and desired controllability upon a shot with a short iron are achieved. In this respect, the hardness Hc is more preferably less than the hardness Hm2 of the outer mid layer 8.

When the golf ball 2 is hit, the cover 12 including the polyurethane absorbs the shock. This absorption achieves soft feel at impact. Particularly, when the golf ball 2 is hit with a short iron or a putter, the cover 12 achieves excellent feel at impact.

In light of achievement of both desired flight performance and desired controllability, the difference (Hm1-Hc) between the hardness Hm1 of the inner mid layer 6 and the hardness Hc of the cover 12 is preferably equal to or greater than 30, more preferably equal to or greater than 33, and particularly preferably equal to or greater than 35. The difference (Hm1-Hc) is preferably equal to or less than 45 and particularly preferably equal to or less than 40. In the golf ball 2 in which the hardness of the inner mid layer 6 and the hardness of the cover 12 meet this condition, a spin rate is suppressed upon a shot with a driver. In the golf ball 2, a backspin rate is high upon an approach shot.

Furthermore, in light of achievement of both desired flight performance and desired controllability, the difference (Hm2-Hc) between the hardness Hm2 of the outer mid layer 8 and the hardness Hc of the cover 12 is preferably equal to or greater than 10 and particularly preferably equal to or greater than 18. The difference (Hm2-Hc) is preferably equal to or less than 30.

The cover 12 preferably has a JIS-C hardness less than the surface hardness Hs of the core 4. When the golf ball 2 is hit with a short iron, the flexible cover 12 is squeezed between the hard core 4 and the hard clubface. This squeeze suppresses a slip of the golf ball 2 relative to the clubface. Due to the suppression of the slip, a high spin rate is obtained. The suppression of the slip suppresses variation of a spin rate. In light of suppression of a slip, the difference between the surface hardness Hs of the core 4 and the JIS-C hardness of the cover 12 is preferably equal to or greater than 30 and particularly preferably equal to or greater than 40.

In light of flight performance upon a shot with a driver, the cover 12 has a thickness Tc of preferably 0.8 mm or less and more preferably 0.6 mm or less. In light of durability and controllability, the thickness Tc is preferably equal to or greater than 0.3 mm and particularly preferably equal to or greater than 0.5 mm.

For forming the cover 12, known methods such as injection molding, compression molding, and the like can be used. When forming the cover 12, the dimples 14 are formed by pimples formed on the cavity face of a mold.

In light of achievement of both desired flight performance and desired controllability, the principal component of the base resin of the resin composition of the cover 12 is preferably a urethane resin or a urea resin, and the principal component of the base resin of the resin composition of the outer mid layer 8 is preferably an ionomer resin. In other words, the principal component of the base resin of the outer mid layer 8 is different from the principal component of the base resin of the cover 12.

In light of durability, the golf ball 2 that further includes the reinforcing layer 10 between the outer mid layer 8 and the cover 12 is preferred. The reinforcing layer 10 is positioned between the outer mid layer 8 and the cover 12. The reinforcing layer 10 firmly adheres to the outer mid layer 8 and also to the cover 12. The reinforcing layer 10 suppresses separation of the cover 12 from the outer mid layer 8. As described above, the cover 12 of the golf ball 2 is thin. When the golf ball 2 is hit by the edge of a clubface, a wrinkle is likely to occur. The reinforcing layer 10 suppresses occurrence of a wrinkle to improve the durability of the golf ball 2.

As the base polymer of the reinforcing layer 10, a two-component curing type thermosetting resin is suitably used. Specific examples of two-component curing type thermosetting resins include epoxy resins, urethane resins, acrylic resins, polyester resins, and cellulose resins. In light of strength and durability of the reinforcing layer 10, two-component curing type epoxy resins and two-component curing type urethane resins are preferred.

A two-component curing type epoxy resin is obtained by curing an epoxy resin with a polyamide type curing agent. Examples of epoxy resins used in two-component curing type epoxy resins include bisphenol A type epoxy resins, bisphenol F type epoxy resins, and bisphenol AD type epoxy resins. A bisphenol A type epoxy resin is obtained by a reaction of bisphenol A and an epoxy group-containing compound such as epichlorohydrin or the like. A bisphenol F type epoxy resin is obtained by a reaction of bisphenol F and an epoxy group-containing compound. A bisphenol AD type epoxy resin is obtained by a reaction of bisphenol AD and an epoxy group-containing compound. In light of balance among flexibility, chemical resistance, heat resistance, and toughness, bisphenol A type epoxy resins are preferred.

The polyamide type curing agent has a plurality of amino groups and one or more amide groups . The amino groups can react with epoxy groups. Specific examples of the polyamide type curing agent include polyamide amine curing agents and modified products thereof. A polyamide amine curing agent is obtained by a condensation reaction of a polymerized fatty acid and a polyamine. A typical polymerized fatty acid is obtained by heating and combining natural fatty acids including a large amount of unsaturated fatty acids, such as linoleic acid, linolenic acid, and the like, in the presence of a catalyst. Specific examples of unsaturated fatty acids include tall oil, soybean oil, linseed oil, and fish oil. A hydrogenated polymerized fatty acid having a dimer content of 90% by weight or greater and a trimer content of 10% by weight or less is preferred. Examples of preferable polyamines include polyethylene diamines, polyoxyalkylene diamines, and derivatives thereof.

In a mixture of an epoxy resin and a polyamide type curing agent, the ratio of the epoxy equivalent of the epoxy resin to the amine active hydrogen equivalent of the polyamide type curing agent is preferably equal to or greater than 1.0/1.4 but equal to or less than 1.0/1.0.

A two-component curing type urethane resin is obtained by a reaction of a base material and a curing agent. A two-component curing type urethane resin obtained by a reaction of a base material containing a polyol component and a curing agent containing a polyisocyanate or a derivative thereof, and a two-component curing type urethane resin obtained by a reaction of a base material containing an isocyanate group-terminated urethane prepolymer and a curing agent having active hydrogen, can be used. Particularly, a two-component curing type urethane resin obtained by a reaction of a base material containing a polyol component and a curing agent containing a polyisocyanate or a derivative thereof, is preferred.

As the polyol component of the base material, a urethane polyol is preferably used. The urethane polyol has urethane bonds and at least two or more hydroxyl groups. Preferably, the urethane polyol has hydroxyl groups at its ends. The urethane polyol can be obtained by causing a reaction of a polyol and a polyisocyanate at such a ratio that the hydroxyl groups of the polyol component are excessive in mole ratio with respect to the isocyanate groups of the polyisocyanate.

The polyol used for producing the urethane polyol has a plurality of hydroxyl groups. Polyols having a weight average molecular weight of 50 or greater but 2000 or less are preferred, and polyols having a weight average molecular weight of 100 or greater but 1000 or less are particularly preferred. Examples of low-molecular-weight polyols include diols and triols. Specific examples of diols include ethylene glycol, diethylene glycol, triethylene glycol, 1,3-butanediol, 1,4-butanediol, neopentyl glycol, and 1,6-hexanediol. Specific examples of triols include trimethylol propane and hexanetriol. Examples of high-molecular-weight polyols include polyether polyols such as polyoxyethylene glycol (PEG), polyoxypropylene glycol (PPG), and polyoxytetramethylene glycol (PTMG); condensed polyester polyols such as polyethylene adipate (PEA), polybutylene adipate (PBA), and polyhexamethylene adipate (PHMA) ; lactone polyester polyols such as poly-ε-caprolactone (PCL); polycarbonate polyols such as polyhexamethylene carbonate; and acrylic polyols. Two or more polyols may be used in combination.

The polyisocyanate used for producing the urethane polyol has a plurality of isocyanate groups. Specific examples of the polyisocyanate include aromatic polyisocyanates such as 2,4-toluene diisocyanate, 2,6-toluene diisocyanate, a mixture (TDI) of 2,4-toluene diisocyanate and 2,6-toluene diisocyanate, 4,4'-diphenylmethane diisocyanate (MDI), 1,5-naphthylene diisocyanate (NDI), 3,3'-bitolylene-4,4'-diisocyanate (TODI), xylylene diisocyanate (XDI), tetramethylxylylene diisocyanate (TMXDI), and paraphenylene diisocyanate (PPDI); alicyclic polyisocyanates such as 4,4'-dicyclohexylmethane diisocyanate (H₁₂MDI), hydrogenated xylylene diisocyanate (H₆XDI), and isophorone diisocyanate (IPDI); and aliphatic polyisocyanates such as hexamethylene diisocyanate (HDI) . Two or more of these polyisocyanates may be used in combination. In light of weather resistance, TMXDI, XDI, HDI, H₆XDI, IPDI, and H₁₂MDI are preferred.

In the reaction of the polyol and the polyisocyanate for producing the urethane polyol, a known catalyst can be used. A typical catalyst is dibutyl tin dilaurate.

In light of strength of the reinforcing layer 10, the proportion of the urethane bonds included in the urethane polyol is preferably equal to or greater than 0.1 mmol/g. In light of followability of the reinforcing layer 10 to the cover 12, the proportion of the urethane bonds included in the urethane polyol is preferably equal to or less than 5 mmol/g. The proportion of the urethane bonds can be adjusted by adjusting the molecular weight of the polyol, which is the material for the urethane polyol, and adjusting the blending ratio of the polyol and the polyisocyanate.

From the standpoint that the time taken for the reaction of the base material and the curing agent is short, the weight average molecular weight of the urethane polyol is preferably equal to or greater than 4000 and particularly preferably equal to or greater than 4500. In light of adhesion of the reinforcing layer 10, the weight average molecular weight of the urethane polyol is preferably equal to or less than 10000 and particularly preferably equal to or less than 9000.

In light of adhesion of the reinforcing layer 10, the hydroxyl value (mg KOH/g) of the urethane polyol is preferably equal to or greater than 15 and particularly preferably equal to or greater than 73. From the standpoint that the time taken for the reaction of the base material and the curing agent is short, the hydroxyl value of the urethane polyol is preferably equal to or less than 130 and particularly preferably equal to or less than 120.

The base material may contain, together with a urethane polyol, a polyol that does not have any urethane bond. The aforementioned polyol that is the material for the urethane polyol can be used in the base material. Polyols compatible with the urethane polyol are preferred. From the standpoint that the time taken for the reaction of the base material and the curing agent is short, the proportion of the urethane polyol in the base material on the solid content basis is preferably equal to or greater than 50% by weight and particularly preferably equal to or greater than 80% by weight. Ideally, the proportion is 100% by weight.

The curing agent contains a polyisocyanate or a derivative thereof. The aforementioned polyisocyanate that is the material for the urethane polyol can be used in the curing agent.

The reinforcing layer 10 may include additives such as a coloring agent (typically, titanium dioxide), a phosphate-based stabilizer, an antioxidant, a light stabilizer, a fluorescent brightener, an ultraviolet absorber, an anti-blocking agent, and the like. The additives may be added to the base material of the two-component curing type thermosetting resin, or may be added to the curing agent of the two-component curing type thermosetting resin.

The reinforcing layer 10 is obtained by applying, to the surface of the outer mid layer 8, a liquid that is prepared by dissolving or dispersing the base material and the curing agent in a solvent. In light of workability, application with a spray gun is preferred. After the application, the solvent is volatilized to permit a reaction of the base material with the curing agent, thereby forming the reinforcing layer 10. Examples of preferable solvents include toluene, isopropyl alcohol, xylene, methyl ethyl ketone, methyl isobutyl ketone, ethylene glycol monomethyl ether, ethylbenzene, propylene glycol monomethyl ether, isobutyl alcohol, and ethyl acetate.

In light of feel at impact, the golf ball 2 has an amount of compressive deformation Db of preferably 2.1 mm or greater, more preferably 2.2 mm or greater, and particularly preferably 2.3 mm or greater. In light of resilience performance, the amount of compressive deformation Db is preferably equal to or less than 3.2 mm, more preferably equal to or less than 3.0 mm, and particularly preferably equal to or less than 2.8 mm.

For measurement of the amount of compressive deformation, a YAMADA type compression tester is used. In the tester, a sphere (the golf ball 2, the core 4, or the like) is placed on a hard plate made of metal. Next, a cylinder made of metal gradually descends toward the sphere. The sphere, squeezed between the bottom face of the cylinder and the hard plate, becomes deformed. A migration distance of the cylinder, starting from the state in which an initial load of 98 N is applied to the sphere up to the state in which a final load of 1274 N is applied thereto, is measured.

### [Second Embodiment]

A golf ball 102 shown in FIG. 3 includes a spherical core 104, an inner mid layer 106 positioned outside the core 104, an outer mid layer 108 positioned outside the inner mid layer 106, a reinforcing layer 110 positioned outside the outer mid layer 108, and a cover 112 positioned outside the reinforcing layer 110. On the surface of the cover 112, a large number of dimples 114 are formed. Of the surface of the golf ball 102, a part other than the dimples 114 is a land 116. The golf ball 102 includes a paint layer and a mark layer on the external side of the cover 112, but these layers are not shown in the drawing.

The golf ball 102 has a diameter of 40 mm or greater but 45 mm or less. From the standpoint of conformity to the rules established by the United States Golf Association (USGA), the diameter is preferably equal to or greater than 42.67 mm. In light of suppression of air resistance, the diameter is preferably equal to or less than 44 mm and more preferably equal to or less than 42.80 mm. The golf ball 102 has a weight of 40 g or greater but 50 g or less. In light of attainment of great inertia, the weight is preferably equal to or greater than 44 g and more preferably equal to or greater than 45.00 g. From the standpoint of conformity to the rules established by the USGA, the weight is preferably equal to or less than 45.93 g.

FIG. 4 is a line graph showing a hardness distribution of the core 104 of the golf ball 102 in FIG. 3 according to the present invention. The horizontal axis of the graph indicates the ratio (%) of a distance from the central point of the core 104 to the radius of the core 104. The vertical axis of the graph indicates a JIS-C hardness. Nine measuring points obtained by dividing a region from the central point of the core 104 to the surface of the core 104 at intervals of 12.5% of the radius of the core 104 are plotted in the graph. The ratio of the distance from the central point of the core 104 to each of these measuring points to the radius of the core 104 is as follows.
First point: 0.0% (central point)
Second point: 12.5%
Third point: 25.0%
Fourth point: 37.5%
Fifth point: 50.0%
Sixth point: 62.5%
Seventh point: 75.0%
Eighth point: 87.5%
Ninth point: 100.0% (surface)

Hardnesses at the first to eighth points are measured by pressing a JIS-C type hardness scale against a cut plane of the core 104 that has been cut into two halves. A hardness at the ninth point is measured by pressing the JIS-C type hardness scale against the surface of the spherical core 104. For the measurement, an automated rubber hardness measurement machine (trade name "P1", manufactured by Kobunshi Keiki Co., Ltd.), to which this hardness scale is mounted, is used.

FIG. 4 also shows a linear approximation curve obtained by a least-square method on the basis of the distances and the hardnesses of the nine measuring points. In FIG. 4, the broken line does not greatly deviate from the linear approximation curve. In other words, the broken line has a shape close to the linear approximation curve. That is, in the core 104 according to the present invention, the hardness linearly increases from its central point toward its surface. When the golf ball 102 that includes the core 104 is hit with a driver, the energy loss is low. The core 104 has excellent resilience performance. When the golf ball 102 is hit with a driver, the flight distance is large. In the core 104, the hardness continuously increases from its central point toward its surface. In the core 104, there is no discontinuous point caused by a multilayer structure. When the golf ball 102 that includes the core 104 deforms by being hit, no local load is applied thereto. The golf ball 102 has excellent durability.

In the core 104, R² of the linear approximation curve obtained by the least-square method is equal to or greater than 0.95. R² is an index indicating the linearity of the broken line. For the core 104 for which R² is equal to or greater than 0.95, the shape of the broken line of the hardness distribution is close to a straight line. The core 104 for which R² is equal to or greater than 0.95 has excellent resilience performance. In this respect, R² is more preferably equal to or greater than 0.97 and particularly preferably equal to or greater than 0.99. R² is calculated by squaring a correlation coefficient R. The correlation coefficient R is calculated by dividing the covariance of the distance (%) from the central point and the hardness (JIS-C) by the standard deviation of the distance (%) from the central point and the standard deviation of the hardness (JIS-C) .

The core 104 is obtained by crosslinking a rubber composition. The rubber composition includes:
(a) a base rubber;
(b) a co-crosslinking agent;
(c) a crosslinking initiator; and
(d) an acid and/or a salt.

The rubber composition of the core 104 can include the base rubber (a) described above for the core 4 of the first embodiment.

The co-crosslinking agent (b) is:
(b1) an α, β-unsaturated carboxylic acid having 3 to 8 carbon atoms; and/or
(b2) a metal salt of an α,β-unsaturated carboxylic acid having 3 to 8 carbon atoms.
The rubber composition of the core 104 can include the co-crosslinking agent (b) described above for the core 4 of the first embodiment.

The metal salt (b2) of the α,β-unsaturated carboxylic acid graft-polymerizes with the molecular chain of the base rubber, thereby crosslinking the rubber molecules. When the rubber composition includes the α,β-unsaturated carboxylic acid (b1), the rubber composition preferably further includes a metal compound (e). The metal compound (e) reacts with the α,β-unsaturated carboxylic acid (b1) in the rubber composition. A salt obtained by this reaction graft-polymerizes with the molecular chain of the base rubber. The rubber composition of the core 104 can include the metal compound (e) described above for the core 4 of the first embodiment.

In light of resilience performance of the golf ball 102, the amount of the co-crosslinking agent (b) is preferably equal to or greater than 15 parts by weight and particularly preferably equal to or greater than 20 parts by weight, per 100 parts by weight of the base rubber. In light of feel at impact, the amount is preferably equal to or less than 50 parts by weight, more preferably equal to or less than 45 parts by weight, and particularly preferably equal to or less than 40 parts by weight, per 100 parts by weight of the base rubber.

The rubber composition of the core 104 can include the crosslinking initiator (c) described above for the core 4 of the first embodiment. In light of resilience performance of the golf ball 102, the amount of the crosslinking initiator (c) is preferably equal to or greater than 0.2 parts by weight and particularly preferably equal to or greater than 0.5 parts by weight, per 100 parts by weight of the base rubber. In light of feel at impact and durability of the golf ball 102, the amount is preferably equal to or less than 5 parts by weight and particularly preferably equal to or less than 2.5 parts by weight, per 100 parts by weight of the base rubber.

The rubber composition of the core 104 can include the acid and/or the salt (d) described above for the core 4 of the first embodiment. The acid component included in the acid and/or the salt (d) has reactivity with a cationic component. During heating and forming of the core 104, the acid dissociates and reacts with the cationic component of the co-crosslinking agent (b). It is thought that the acid inhibits formation of the metal crosslinks by the co-crosslinking agent (b) in the central portion of the core 104. The acid component included in the salt exchanges the cationic component with the co-crosslinking agent (b). It is inferred that during heating and forming of the core 104, the salt breaks the metal crosslinks by the co-crosslinking agent (b) in the central portion of the core 104. In the present invention, the co-crosslinking agent (b) is not included in the concept of the acid and/or the salt (d) .

From the standpoint that the hardness distribution of the core 104 is made appropriate, the amount of the acid and/or the salt (d) is preferably equal to or greater than 1.0 parts by weight, more preferably equal to or greater than 1.5 parts by weight, and even more preferably equal to or greater than 2 parts by weight, per 100 parts by weight of the base rubber. In light of resilience performance, the amount is preferably equal to or less than 40 parts by weight, more preferably equal to or less than 30 parts by weight, and particularly preferably equal to or less than 20 parts by weight, per 100 parts by weight of the base rubber.

The weight ratio of the co-crosslinking agent (b) and the acid and/or the salt (d) in the rubber composition is preferably equal to or greater than 3/7 but equal to or less than 9/1, and is particularly preferably equal to or greater than 4/6 but equal to or less than 8/2. From the rubber composition in which this weight ratio is within the above range, the core 104 whose hardness linearly increases from its central point toward its surface is obtained.

As the co-crosslinking agent (b), zinc acrylate is preferably used. Zinc acrylate whose surface is coated with stearic acid or zinc stearate for the purpose of improving dispersibility to rubber is present. When the rubber composition includes this zinc acrylate, the stearic acid or zinc stearate coating the zinc acrylate is not included in the concept of the acid and/or the salt (d).

The rubber composition of the core 104 preferably further includes the organic sulfur compound (f) described above for the core 4 of the first embodiment. The organic sulfur compound (f) can contribute to control of: the linearity of the hardness distribution of the core 104; and the degree of an outer-hard/inner-soft structure.

From the standpoint that the hardness distribution of the core 104 is made appropriate, the amount of the organic sulfur compound (f) is preferably equal to or greater than 0.05 parts by weight, more preferably equal to or greater than 0.1 parts by weight, and particularly preferably equal to or greater than 0.2 parts by weight, per 100 parts by weight of the base rubber. In light of resilience performance, the amount is preferably equal to or less than 5 parts by weight, more preferably equal to or less than 3 parts by weight, and particularly preferably equal to or less than 1 parts by weight, per 100 parts by weight of the base rubber.

For the purpose of adjusting specific gravity and the like, a filler may be included in the core 104. Examples of suitable fillers include zinc oxide, barium sulfate, calcium carbonate, and magnesium carbonate . The amount of the filler is determined as appropriate so that the intended specific gravity of the core 104 is accomplished. A particularly preferable filler is zinc oxide. Zinc oxide serves not only as a specific gravity adjuster but also as a crosslinking activator.

According to need, an anti-aging agent, a coloring agent, a plasticizer, a dispersant, sulfur, a vulcanization accelerator, and the like are added to the rubber composition of the core 104. Crosslinked rubber powder or synthetic resin powder may also be dispersed in the rubber composition.

During heating and forming of the core 104, the heat of the crosslinking reaction of the base rubber remains near the central point of the core 104. Thus, during heating and forming of the core 104, the temperature at the central portion is high. The temperature gradually decreases from the central point toward the surface. The acid and/or the salt (d) reacts with a metal salt of the co-crosslinking agent (b) to break metal crosslinks. This reaction is accelerated in a region where the temperature is high. In other words, breaking of the metal crosslinks is likely to occur in the central portion of the core 104 where the temperature is high, and is unlikely to occur near the surface of the core 104. As a result, the crosslinking density of the core 104 increases from its central point toward its surface. In the core 104, the hardness linearly increases from its central point toward its surf ace. Further, since the rubber composition includes the organic sulfur compound (f) together with the acid and/or the salt (d), the gradient of the hardness distribution can be controlled, and the degree of the outer-hard/inner-soft structure of the core 104 can be increased.

In the present invention, a JIS-C hardness at a measuring point whose ratio of the distance from the central point of the core 104 to the radius of the core 104 is x% is represented by H(x). The hardness at the central point of the core 104 is represented by H(0.0). The surface hardness of the core 104 is represented by Hs. The difference (Hs-H(0.0)) between the surface hardness Hs and the central hardness H(0.0) is equal to or greater than 15. The difference is great. In other words, the core 104 has an outer-hard/inner-soft structure. When the core 104 is hit with a driver, the recoil (torsional return) is great, and thus spin is suppressed. The core 104 contributes to the flight performance of the golf ball 102. In light of flight performance, the difference (Hs-H(0.0)) is more preferably equal to or greater than 25 and particularly preferably equal to or greater than 30. From the standpoint that the core 104 can easily be formed, the difference (Hs-H (0.0)) is preferably equal to or less than 50.

The hardness H(0.0) at the central point of the core 104 is preferably equal to or greater than 40 but equal to or less than 70. The golf ball 102 that includes the core 104 having a hardness H(0.0) of 40 or greater has excellent resilience performance. The hardness H(0.0) is more preferably equal to or greater than 45 and particularly preferably equal to or greater than 50. In the core 104 having a hardness H(0.0) of 70 or less, an outer-hard/inner-soft structure can be achieved. In the golf ball 102 that includes the core 104, spin can be suppressed. The hardness H(0.0) is more preferably equal to or less than 68 and particularly preferably equal to or less than 65.

The hardness Hs at the surface of the core 104 is preferably equal to or greater than 78 but equal to or less than 96. In the core 104 having a hardness Hs of 78 or greater, an outer-hard/inner-soft structure can be achieved. In the golf ball 102 that includes the core 104, spin can be suppressed. The hardness Hs is more preferably equal to or greater than 80 and particularly preferably equal to or greater than 82. The golf ball 102 that includes the core 104 having a hardness Hs of 96 or less has excellent durability. The hardness Hs is more preferably equal to or less than 94 and particularly preferably equal to or less than 92.

The core 104 has a diameter of 36.0 mm or greater. The core 104 having a diameter of 36.0 mm or greater can achieve excellent resilience performance of the golf ball 102. The core 104 having a diameter of 36.0 mm or greater can achieve an outer-hard/inner-soft structure of the golf ball 102. In this respect, the diameter is preferably equal to or greater than 37.0 mm and particularly preferably equal to or greater than 38.0 mm. Furthermore, the diameter of the core 104 is preferably equal to or less than 40.0 mm. In the golf ball 102 that includes the core 104 having a diameter of 40.0 mm or less, the inner mid layer 106, the outer mid layer 108, and the cover 112 can have sufficient thicknesses. The golf ball 102 that includes the inner mid layer 106, the outer mid layer 108, and the cover 112 which have large thicknesses has excellent durability. In this respect, the diameter is particularly preferably equal to or less than 39.0 mm.

In light of feel at impact, the core 104 has an amount of compressive deformation Dc of preferably 3.0 mm or greater and particularly preferably 3.2 mm or greater. In light of resilience performance, the amount of compressive deformation Dc is preferably equal to or less than 3.8 mm and particularly preferably equal to or less than 3.5 mm.

For the inner mid layer 106, a resin composition is suitably used. Examples of the base resin of the resin composition include ionomer resins, polystyrenes, polyesters, polyamides, and polyolefins.

Particularly preferable base resins are ionomer resins. The golf ball 102 that includes the inner mid layer 106 including an ionomer resin has excellent resilience performance. An ionomer resin and another resin may be used in combination for the inner mid layer 106. In this case, the principal component of the base resin is preferably the ionomer resin. Specifically, the proportion of the ionomer resin to the entire base resin is preferably equal to or greater than 40% by weight, more preferably equal to or greater than 60% by weight, and particularly preferably equal to or greater than 70% by weight.

The inner mid layer 106 can include the ionomer resin described above for the golf ball 2 of the first embodiment. The inner mid layer 106 can include the styrene block-containing thermoplastic elastomer described above for the golf ball 2 of the first embodiment.

According to need, a coloring agent such as titanium dioxide, a filler such as barium sulfate, a dispersant, an antioxidant, an ultraviolet absorber, a light stabilizer, a fluorescent material, a fluorescent brightener, and the like are included in the resin composition of the inner mid layer 106 in an adequate amount.

In light of flight performance, the inner mid layer 106 has a Shore D hardness Hm1 of preferably 30 or greater and more preferably 40 or greater. In the golf ball 102 that includes the inner mid layer 106 having a hardness Hm1 in this range, a spin rate is sufficiently suppressed upon a shot with a driver. The flight distance of the golf ball 102 is large. In light of controllability of the golf ball 102, the hardness Hm1 is preferably less than 50 and particularly preferably equal to or less than 47. When the golf ball 102 is hit with a short iron, the spin rate is high.

The Shore D hardness Hm1 of the inner mid layer 106 is measured according to the standards of "ASTM-D 2240-68" with a Shore D type hardness scale mounted to an automated rubber hardness measurement machine (trade name "P1", manufactured by Kobunshi Keiki Co., Ltd.). For the measurement, a slab that is formed by hot press and that has a thickness of about 2 mm is used. A slab kept at 23°C for two weeks is used for the measurement. At the measurement, three slabs are stacked. A slab formed from the same resin composition as the resin composition of the inner mid layer 106 is used.

The inner mid layer 106 preferably has a thickness T1 of 0.5 mm or greater but 1.6 mm or less. In light of durability, the thickness T1 is more preferably equal to or greater than 0.7 mm. In light of resilience performance, the thickness T1 is more preferably equal to or less than 1.2 mm.

For the outer mid layer 108, a resin composition is suitably used. Examples of the base resin of the resin composition include ionomer resins, polystyrenes, polyesters, polyamides, and polyolefins.

Particularly preferable base resins are ionomer resins. The golf ball 102 that includes the outer mid layer 108 including an ionomer resin has excellent resilience performance. An ionomer resin and another resin may be used in combination for the outer mid layer 108. In this case, the principal component of the base resin is preferably the ionomer resin. Specifically, the proportion of the ionomer resin to the entire base resin is preferably equal to or greater than 50% by weight, more preferably equal to or greater than 60% by weight, and particularly preferably equal to or greater than 70% by weight. The ionomer resin described above for the golf ball 2 of the first embodiment can also be used for the outer mid layer 108. The styrene block-containing thermoplastic elastomer described above for the golf ball 2 of the first embodiment may be used in combination for the outer mid layer 108.

As described later, the outer mid layer 108 has a hardness Hm2 greater than the hardness Hm1 of the inner mid layer 106. By decreasing the amount of the styrene block-containing thermoplastic elastomer included in the resin composition of the outer mid layer 108, a great hardness Hm2 can be achieved. By increasing the amount of a highly elastic resin in the resin composition, a great hardness Hm2 may be achieved. Specific examples of the highly elastic resin include polyamides.

According to need, a coloring agent such as titanium dioxide, a filler such as barium sulfate, a dispersant, an antioxidant, an ultraviolet absorber, a light stabilizer, a fluorescent material, a fluorescent brightener, and the like are included in the resin composition of the outer mid layer 108 in an adequate amount.

From the standpoint that an outer-hard/inner-soft structure is achieved in the sphere consisting of the core 104, the inner mid layer 106, and the outer mid layer 108, the outer mid layer 108 has a Shore D hardness Hm2 of preferably 55 or greater and more preferably 60 or greater. When the golf ball 102 is hit with a driver, the spin rate is low. The flight distance of the golf ball 102 is large. In light of controllability of the golf ball 102, the hardness Hm2 is preferably equal to or less than 70 and particularly preferably equal to or less than 68. When the golf ball 102 is hit with a short iron, the spin rate is high. The hardness Hm2 is measured by the same measurement method as that for the hardness Hm1.

From the standpoint that an outer-hard/inner-soft structure is achieved in the sphere consisting of the core 104, the inner mid layer 106, and the outer mid layer 108, the hardness Hm2 of the outer mid layer 108 is preferably greater than the hardness Hm1 of the inner mid layer 106. When the golf ball 102 that includes the sphere is hit with a driver, the spin rate is low. The flight distance of the golf ball 102 is large.

In light of resilience performance and controllability, the difference (Hm2-Hm1) between the hardness Hm2 of the outer mid layer 108 and the hardness Hm1 of the inner mid layer 106 is preferably equal to or greater than 10 and particularly preferably equal to or greater than 14. In light of flight performance, the difference (Hm2-Hm1) is preferably equal to or less than 30. When the golf ball 102 that includes the inner mid layer 106 and the outer mid layer 108 which have hardnesses in this range is hit with a driver, the spin rate is low. The flight distance of the golf ball 102 is large. When the golf ball 102 is hit with a short iron, the spin rate is high.

The outer mid layer 108 preferably has a thickness T2 of 0.5 mm or greater. In the golf ball 102 that includes the outer mid layer 108 having a thickness T2 of 0.5 mm or greater, the shock by a hit is alleviated. Thus, the golf ball 2 has excellent durability. In this respect, the thickness T2 is more preferably equal to or greater than 0.7 mm. The thickness T2 is preferably equal to or less than 1.6 mm. The golf ball 102 that includes the outer mid layer 108 having a thickness T2 of 1.6 mm or less includes a relatively large core 104. The golf ball 102 exerts sufficient resilience performance. In this respect, the thickness T2 is particularly preferably equal to or less than 1.2 mm.

The sum (T1+T2) of the thickness T1 and the thickness T2 is preferably equal to or greater than 1.0 mm. In the golf ball 102, the shock by a hit is alleviated. Thus, the golf ball 102 has excellent durability. In this respect, the sum (T1+T2) is more preferably equal to or greater than 1.3 mm. The sum (T1+T2) is preferably equal to or less than 3.0 mm. The golf ball 102 includes a relatively large core 104. The golf ball 102 exerts sufficient resilience performance. In this respect, the sum (T1+T2) is more preferably equal to or less than 2.0 mm.

For forming the outer mid layer 108, known methods such as injection molding, compression molding, and the like can be used.

For the cover 112, a resin composition is suitably used. A preferable base resin of the resin composition is a urethane resin or a urea resin. The principal component of the urethane resin is a polyurethane. The polyurethane is flexible. When the golf ball 102 that includes the cover 112 formed from the resin composition that includes the polyurethane is hit with a short iron, the spin rate is high. The cover 112 formed from this resin composition contributes to controllability upon a shot with a short iron. The polyurethane also contributes to the scuff resistance of the cover 112. Furthermore, the polyurethane can also contribute to excellent feel at impact when the golf ball 102 is hit with a putter or a short iron.

In light of ease of forming the cover 112, a preferable base resin is a thermoplastic polyurethane elastomer. The cover 112 can include the thermoplastic polyurethane elastomer described above for the golf ball 2 of the first embodiment. A thermoplastic polyurethane elastomer and another resin may be used in combination. Examples of the resin that can be used in combination include thermoplastic polyester elastomers, thermoplastic polyamide elastomers, thermoplastic polyolefin elastomers, styreneblock-containing thermoplastic elastomers, and ionomer resins. When a thermoplastic polyurethane elastomer and another resin are used in combination, the thermoplastic polyurethane elastomer is included as the principal component of the base polymer, in light of spin performance and scuff resistance. The proportion of the thermoplastic polyurethane elastomer to the entire base polymer is preferably equal to or greater than 50% by weight, more preferably equal to or greater than 70% by weight, and particularly preferably equal to or greater than 85% by weight.

According to need, a coloring agent such as titanium dioxide, a filler such as barium sulfate, a dispersant, an antioxidant, an ultraviolet absorber, a light stabilizer, a fluorescent material, a fluorescent brightener, and the like are included in the cover 112 in an adequate amount.

The cover 112 preferably has a Shore D hardness Hc of 48 or less. The golf ball 102 that includes the cover 112 having a hardness Hc of 48 or less has excellent controllability. In this respect, the hardness Hc is more preferably equal to or less than 40 and particularly preferably equal to or less than 32. In light of flight distance upon a shot with a driver, the hardness Hc is preferably equal to or greater than 10, more preferably equal to or greater than 15, and particularly preferably equal to or greater than 20. The hardness Hc is measured by the same measurement method as that for the hardness Hm1.

The hardness Hc of the cover 112 is less than the hardness Hm2 of the outer mid layer 108. When the golf ball 102 is hit with a driver, the sphere consisting of the core 104, the inner mid layer 106, and the outer mid layer 108 becomes significantly distorted since the head speed is high. Since this sphere has an outer-hard/inner-soft structure, the spin rate is suppressed. The hardness of the core 104 linearly changes. Thus, the golf ball 102 is launched at a high speed due to deformation and restoration of the core 104. The suppression of the spin rate and the high launch speed achieve a large flight distance. When the golf ball 102 is hit with a short iron, this sphere becomes less distorted since the head speed is low. When the golf ball 102 is hit with a short iron, the behavior of the golf ball 102 mainly depends on the cover 112. Since the cover 112 is flexible, a slip between the golf ball 102 and a clubface is suppressed. Due to the suppression of the slip, a high spin rate is obtained. The high spin rate achieves excellent controllability. In the golf ball 102, both desired flight performance upon a shot with a driver and desired controllability upon a shot with a short iron are achieved. In this respect, the hardness Hc is more preferably less than the hardness Hm1 of the inner mid layer 106.

When the golf ball 102 is hit, the cover 112 including the polyurethane absorbs the shock. This absorption achieves soft feel at impact. Particularly, when the golf ball 102 is hit with a short iron or a putter, the cover 112 achieves excellent feel at impact.

In light of achievement of both desired flight performance and desired controllability, the difference (Hm2-Hc) between the hardness Hm2 of the outer mid layer 108 and the hardness Hc of the cover 112 is preferably equal to or greater than 30, more preferably equal to or greater than 33, and particularly preferably equal to or greater than 36. The difference (Hm2-Hc) is preferably equal to or less than 45 and particularly preferably equal to or less than 40. In the golf ball 102 in which the hardness of the outer mid layer 108 and the hardness of the cover 112 meet this condition, a backspin rate is suppressed upon a shot with a driver. In the golf ball 102, a backspin rate is high upon an approach shot.

In light of achievement of both desired flight performance and desired controllability, the difference (Hm1-Hc) between the hardness Hm1 of the inner mid layer 106 and the hardness Hc of the cover 112 is preferably equal to or greater than 10 and particularly preferably equal to or greater than 15. The difference (Hm1-Hc) is preferably equal to or less than 22.

The cover 112 preferably has a JIS-C hardness less than the surface hardness Hs of the core 104. When the golf ball 102 is hit with a short iron, the flexible cover 112 is squeezed between the hard core 104 and the hard clubface. This squeeze suppresses a slip of the golf ball 102 relative to the clubface. Due to the suppression of the slip, a high spin rate is obtained. The suppression of the slip suppresses variation of a spin rate. In light of suppression of a slip, the difference between the surface hardness Hs of the core 104 and the JIS-C hardness of the cover 112 is preferably equal to or greater than 20 and particularly preferably equal to or greater than 27.

In light of flight performance upon a shot with a driver, the cover 112 has a thickness Tc of preferably 0.8 mm or less, more preferably 0.6 mm or less, and particularly preferably 0.4 mm or less. In light of durability and controllability, the thickness Tc is preferably equal to or greater than 0.2 mm and particularly preferably equal to or greater than 0.3 mm.

For forming the cover 112, known methods such as injection molding, compression molding, and the like can be used. When forming the cover 112, the dimples 114 are formed by pimples formed on the cavity face of a mold.

In light of achievement of both desired flight performance and desired controllability, the principal component of the base resin of the resin composition of the cover 112 is preferably a urethane resin or a urea resin, and the principal component of the base resin of the resin composition of the outer mid layer 108 is preferably an ionomer resin. In other words, the principal component of the base resin of the outer mid layer 108 is different from the principal component of the base resin of the cover 112.

In light of durability, the golf ball 102 that further includes the reinforcing layer 110 between the outer mid layer 108 and the cover 112 is preferred. The reinforcing layer 110 is positioned between the outer mid layer 108 and the cover 112. The reinforcing layer 110 firmly adheres to the outer mid layer 108 and also to the cover 112. The reinforcing layer 110 suppresses separation of the cover 112 from the outer mid layer 108. As described above, the cover 112 of the golf ball 102 is thin. When the golf ball 102 is hit by the edge of a clubface, a wrinkle is likely to occur. The reinforcing layer 110 suppresses occurrence of a wrinkle to improve the durability of the golf ball 102.

As the base polymer of the reinforcing layer 110, a two-component curing type thermosetting resin is suitably used. The reinforcing layer 110 can include the two-component curing type thermosetting resin described above for the golf ball 2 of the first embodiment. The reinforcing layer 110 may include additives such as a coloring agent (typically, titanium dioxide), a phosphate-based stabilizer, an antioxidant, alight stabilizer, a fluorescent brightener, an ultraviolet absorber, an anti-blocking agent, and the like. The additives may be added to the base material of the two-component curing type thermosetting resin, or may be added to the curing agent of the two-component curing type thermosetting resin.

The reinforcing layer 110 is obtained by applying, to the surface of the outer mid layer 108, a liquid that is prepared by dissolving or dispersing the base material and the curing agent in a solvent. In light of workability, application with a spray gun is preferred. After the application, the solvent is volatilized to permit a reaction of the base material with the curing agent, thereby forming the reinforcing layer 110. Examples of preferable solvents include toluene, isopropyl alcohol, xylene, methyl ethyl ketone, methyl isobutyl ketone, ethylene glycol monomethyl ether, ethylbenzene, propylene glycol monomethyl ether, isobutyl alcohol, and ethyl acetate.

In light of feel at impact, the golf ball 102 has an amount of compressive deformation Db of preferably 2.1 mm or greater, more preferably 2.2 mm or greater, and particularly preferably 2.3 mmorgreater. In light of resilience performance, the amount of compressive deformation Db is preferably equal to or less than 3.2 mm, more preferably equal to or less than 3.0 mm, and particularly preferably equal to or less than 2.8 mm. The amount of compressive deformation is measured by the method described above for the golf ball 2 of the first embodiment.

### EXAMPLES

### [Experiment 1]

### [Example 1-1]

A rubber composition was obtained by kneading 100 parts by weight of a high-cis polybutadiene (trade name "BR-730", manufactured by JSR Corporation), 38 parts by weight of zinc diacrylate (trade name "Sanceler SR", manufactured by SANSHIN CHEMICAL INDUSTRY CO., LTD.), 5 parts by weight of zinc oxide, an appropriate amount of barium sulfate, 0.2 parts by weight of 2-thionaphthol, 0.9 parts by weight of dicumyl peroxide (trade name "Percumyl D" manufactured by NOF Corporation), and 2 parts by weight of zinc octoate (a product of Mitsuwa Chemicals Co. , Ltd.). This rubber composition was placed into a mold including upper and lower mold halves each having a hemispherical cavity, and heated at 170°C for 25 minutes to obtain a spherical core with a diameter of 38.5 mm. The amount of barium sulfate was adjusted such that the weight of a golf ball is 45.6 g.

A resin composition was obtained by kneading 55 parts by weight of an ionomer resin (the aforementioned "Surlyn 8945"), 45 parts by weight of another ionomer resin (the aforementioned "Himilan AM7329"), and 3 parts by weight of titanium dioxide with a twin-screw kneading extruder. The extruding conditions were a screw diameter of 45 mm, a screw rotational speed of 200 rpm, screw L/D of 35, and a die temperature of 160 to 230°C. The core was placed into a mold. The resin composition was injected around the core by injection molding to form an inner mid layer with a thickness of 0.8 mm.

A resin composition was obtained by kneading 27 parts by weight of an ionomer resin (the aforementioned "Surlyn 8945"), 45 parts by weight of another ionomer resin (the aforementioned "Himilan AM7329"), 28 parts by weight of a styrene block-containing thermoplastic elastomer (the aforementioned "Rabalon T3221C"), and 3 parts by weight of titanium dioxide with a twin-screw kneading extruder under the above extruding conditions. The sphere consisting of the core and the inner mid layer was placed into a mold. The resin composition was injected around the sphere by injection molding to form an outer mid layer with a thickness of 0.8 mm.

A paint composition (trade name "POLIN 750LE", manufactured by SHINTO PAINT CO., LTD.) including a two-component curing type epoxy resin as a base polymer was prepared. The base material liquid of this paint composition includes 30 parts by weight of a bisphenol A type solid epoxy resin and 70 parts by weight of a solvent. The curing agent liquid of this paint composition includes 40 parts by weight of a modified polyamide amine, 55 parts by weight of a solvent, and 5 parts by weight of titanium dioxide. The weight ratio of the base material liquid to the curing agent liquid is 1/1. This paint composition was applied to the surface of the outer mid layer with an air gun, and kept at 23°C for 12 hours to obtain a reinforcing layer with a thickness of 10 µm.

A resin composition was obtained by kneading 100 parts by weight of a thermoplastic polyurethane elastomer (the aforementioned "Elastollan NY82A"), 0.2 parts by weight of a hindered amine light stabilizer (trade name "TINUVIN 770", manufactured by Ciba Japan K.K.), 4 parts by weight of titanium dioxide, and 0.04 parts by weight of ultramarine blue with a twin-screw kneading extruder under the above extruding conditions. Half shells were formed from this resin composition by compression molding. The sphere consisting of the core, the inner mid layer, the outer mid layer, and the reinforcing layer was covered with two of these half shells. The sphere and the half shells were placed into a final mold that includes upper and lower mold halves each having a hemispherical cavity and that has a large number of pimples on its cavity face. A cover was obtained by compression molding. The thickness of the cover was 0.5 mm. Dimples having a shape that is the inverted shape of the pimples were formed on the cover. The surface of the cover was polished. A clear paint including a two-component curing type polyurethane as a base material was applied to this cover with an air gun, and was dried and cured to obtain a golf ball of Example I-1 with a diameter of 42.7 mm and a weight of 45.6 g.

### [Examples 1-2 to 1-17 and Comparative Examples I-1 to 1-6]

Golf balls of Examples 1-2 to 1-17 and Comparative Examples I-1 to 1-6 were obtained in the same manner as Example I-1, except the specifications of the core, the inner mid layer, the outer mid layer, and the cover were as shown in Tables 1-6 to I-10 below. The composition and hardness of the core are shown in detail in Tables 1-1 to 1-3 below. The compositions and hardnesses of the inner mid layer and the outer mid layer are shown in Table 1-4 below. The composition and hardness of the cover are shown in Table 1-5 below.

### [Hit with Driver (W#1)]

A driver with a titanium head (trade name "XXIO", manufactured by DUNLOP SPORTS CO. LTD., shaft hardness: S, loft angle: 10.0°) was attached to a swing machine manufactured by True Temper Co. A golf ball was hit under the condition of a head speed of 45 m/sec. The spin rate was measured immediately after the hit. Furthermore, the flight distance from the launch point to the stop point was measured. The average value of data obtained by 10 measurements is shown in Tables 1-6 to I-10 below.

### [Hit with Sand Wedge (SW)]

A sand wedge (trade name "XXIO", manufactured by DUNLOP SPORTS CO. LTD., shaft hardness: R, loft angle: 56.0°) was attached to a swing machine manufactured by True Temper Co. A golf ball was hit under the condition of a head speed of 21 m/sec. The backspin rate was measured immediately after the hit. The average value of data obtained by 10 measurements is shown in Tables 1-6 to I-10 below.

### [Durability]

A driver with a titanium head (trade name "XXIO", manufactured by DUNLOP SPORTS CO. LTD., shaft hardness: S, loft angle: 10.0°) was attached to a swing robot M/C manufactured by True Temper Co. A golf ball having been kept at 23°C for 12 hours was used for the measurement. The golf ball was repeatedly hit under the condition of a head speed of 45 m/sec. The number of hits required to break the golf ball was measured. An index of the average value of data obtained for 12 golf balls is shown in Tables 1-6 to 1-10 below. The higher the index is, the more excellent the durability of the golf ball is.

### [Feel at Impact]

A golf player hit golf balls with a driver with a titanium head (trade name "XXIO" , manufactured by DUNLOP SPORTS CO. LTD. , shaft hardness: S, loft angle: 10.0°). The results of evaluation of feel at impact based on the following criteria are shown in Tables 1-6 to I-10 below.
A: very favorable (soft)
B: favorable (soft)
C: slightly poor (slightly hard)
D: poor (hard)

**Table I-1 Composition and Hardness of Core (parts by weight)**

| Type | (1) | (2) | (3) | (4) | (5) |
|---|---|---|---|---|---|
| BR-730 | 100 | 100 | 100 | 100 | 100 |
| Sanceler SR | 34 | 38 | 38 | 38 | 39 |
| ZN-DA90S | - | - | - | - | - |
| Zinc oxide | 5 | 5 | 5 | 5 | 5 |
| Barium sulfate | * | * | * | * | * |
| 2-thionaphthol | 0.2 | 0.2 | 0.2 | 0.2 | 0.2 |
| Bis(pentabromophenyl ) disulfide | - | - | - | - | - |
| Dicumyl peroxide | 0.9 | 0.9 | 0.9 | 0.9 | 0.9 |
| Zinc octoate | - | 0.5 | 2 | 5 | 10 |
| Zinc stearate | - | - | - | - | - |
| Zinc myristate | - | - | - | - | - |
| Amount of acid/salt | 0 | 0.5 | 2 | 5 | 10 |

| Vulcanization conditions | | | | | |
|---|---|---|---|---|---|
| Temperature (°C) | 170 | 170 | 170 | 170 | 170 |
| Time (min) | 25 | 25 | 25 | 25 | 25 |

| Hardness distribution (JIS-C hardness) | | | | | |
|---|---|---|---|---|---|
| H(0.0) | 57.0 | 55.0 | 55.0 | 56.5 | 55.5 |
| H(12.5) | 68.0 | 65.5 | 62.0 | 59.5 | 59.0 |
| H(25.0) | 73.0 | 70.5 | 67.5 | 64.5 | 64.0 |
| H(37.5) | 74.0 | 72.0 | 69.5 | 67.0 | 67.0 |
| H(50.0) | 74.0 | 73.5 | 71.5 | 70.0 | 69.5 |
| H(62.5) | 74.0 | 75.0 | 72.5 | 74.0 | 72.0 |
| H(75.0) | 78.0 | 76.5 | 77.5 | 80.5 | 80.0 |
| H(87.5) | 82.0 | 81.5 | 82.5 | 85.0 | 84.0 |
| Surface hardness Hs | 87.0 | 86.0 | 86.5 | 89.0 | 87.0 |

| | | | | | |
|---|---|---|---|---|---|
| * Appropriate amount | | | | | |

**Table I-2 Composition and Hardness of Core (parts by weight)**

| Type | (6) | (7) | (8) | (9) | (10) |
|---|---|---|---|---|---|
| BR-730 | 100 | 100 | 100 | 100 | 100 |
| Sanceler SR | 40 | 41 | 35 | 36 | 38 |
| ZN-DA90S | - | - | - | - | - |
| Zinc oxide | 5 | 5 | 5 | 5 | 5 |
| Barium sulfate | * | * | * | * | * |
| 2-thionaphthol | 0.2 | 0.2 | 0.2 | 0.2 | 0.2 |
| Bis(pentabromophenyl ) disulfide | - | - | - | - | - |
| Dicumyl peroxide | 0.9 | 0.9 | 0.9 | 0.9 | 0.9 |
| Zinc octoate | 30 | 45 | - | - | - |
| Zinc stearate | - | - | 10 | 20 | - |
| Zinc myristate | - | - | - | - | 5 |
| Amount of acid/salt | 30 | 45 | 10 | 20 | 5 |

| Vulcanization conditions | | | | | |
|---|---|---|---|---|---|
| Temperature (°C) | 170 | 170 | 170 | 170 | 170 |
| Time (min) | 25 | 25 | 25 | 25 | 25 |

| Hardness distribution (JIS-C hardness) | | | | | |
|---|---|---|---|---|---|
| H(0.0) | 53.5 | 64.0 | 57.5 | 56.0 | 57.0 |
| H(12.5) | 58.5 | 68.0 | 61.0 | 59.0 | 60.5 |
| H(25.0) | 61.5 | 69.5 | 65.5 | 62.0 | 65.0 |
| H(37.5) | 65.0 | 71.0 | 68.0 | 65.5 | 68.0 |
| H(50.0) | 68.0 | 71.5 | 70.0 | 69.0 | 70.0 |
| H(62.5) | 70.5 | 72.5 | 71.5 | 71.0 | 72.0 |
| H(75.0) | 73.5 | 73.5 | 81.0 | 80.0 | 80.5 |
| H(87.5) | 76.0 | 76.0 | 85.0 | 82.0 | 85.0 |
| Surface hardness Hs | 81.0 | 77.0 | 89.0 | 86.0 | 89.0 |

| | | | | | |
|---|---|---|---|---|---|
| * Appropriate amount | | | | | |

**Table I-3 Composition and Hardness of Core (parts by weight)**

| Type | (11) | (12) | (13) | (14) | (15) |
|---|---|---|---|---|---|
| BR-730 | 100 | 100 | 100 | 100 | 100 |
| Sanceler SR | 39 | 40 | - | 39 | 37 |
| ZN-DA90S | - | - | 38 | - | - |
| Zinc oxide | 5 | 5 | 5 | 5 | 5 |
| Barium sulfate | * | * | * | * | * |
| 2-thionaphthol | 0.2 | - | 0.2 | 0.2 | 0.2 |
| Bis(pentabromophenyl ) disulfide | - | 0.3 | - | - | - |
| Dicumyl peroxide | 0.9 | 0.9 | 0.9 | 0.9 | 0.9 |
| Zinc octoate | - | 5 | 5 | 5 | 5 |
| Zinc stearate | - | - | - | - | - |
| Zinc myristate | 10 | - | - | - | - |
| Amount of acid/salt | 10 | 5 | 5 | 5 | 5 |

| Vulcanization conditions | | | | | |
|---|---|---|---|---|---|
| Temperature (°C) | 170 | 170 | 170 | 170 | 170 |
| Time (min) | 25 | 25 | 25 | 25 | 25 |

| Hardness distribution (JIS-C hardness) | | | | | |
|---|---|---|---|---|---|
| H(0.0) | 56.0 | 56.5 | 56.5 | 57.0 | 56.0 |
| H(12.5) | 59.5 | 59.5 | 59.5 | 60.0 | 59.0 |
| H(25.0) | 64.5 | 65.0 | 64.5 | 65.0 | 64.0 |
| H(37.5) | 67.5 | 67.0 | 67.0 | 67.5 | 66.5 |
| H(50.0) | 69.5 | 70.0 | 71.0 | 70.5 | 69.5 |
| H(62.5) | 72.0 | 74.0 | 74.0 | 74.5 | 73.5 |
| H(75.0) | 80.5 | 80.0 | 80.5 | 81.0 | 80.0 |
| H(87.5) | 84.5 | 85.0 | 85.0 | 85.5 | 84.5 |
| Surface hardness Hs | 87.5 | 89.0 | 89.0 | 89.5 | 88.5 |

| | | | | | |
|---|---|---|---|---|---|
| * Appropriate amount | | | | | |

The details of the compounds listed in Tables I-1 to 1-3 are as follows.
BR730: a high-cis polybutadiene manufactured by JSR Corporation (cis-1, 4-bond content: 96% by weight, 1, 2-vinyl bond content: 1.3% by weight, Mooney viscosity (ML₁₊₄ (100°C)) : 55, molecular weight distribution (Mw/Mn): 3)
Sanceler SR: zinc diacrylate manufactured by SANSHIN CHEMICAL INDUSTRY CO., LTD. (a product coated with 10% by weight of stearic acid)
ZN-DA90S: zinc diacrylate manufactured by Nihon Jyoryu Kogyo Co., Ltd. (a product coated with 10% by weight of zinc stearate)
Zinc oxide: trade name "Ginrei R" manufactured by Toho Zinc Co., Ltd.
Barium sulfate : trade name "Barium Sulfate BD" manufactured by Sakai Chemical Industry Co., Ltd.
2-thionaphthol: a product of Tokyo Chemical Industry Co. , Ltd.
Bis(pentabromophenyl)disulfide: a product of Kawaguchi Chemical Industry Co., LTD.
Dicumyl peroxide: trade name "Percumyl D" manufactured by NOF Corporation
Zinc octoate: a product of Mitsuwa Chemicals Co., Ltd. (purity: 99% or greater)
Zinc stearate: a product of Wako Pure Chemical Industries, Ltd. (purity: 99% or greater)
Zinc myristate: a product of NOF Corporation (purity: 90% or greater)

**Table I-4 Compositions and Hardnesses of Inner Mid Layer and Outer Mid Layer (parts by weight)**

| Type | a | b | c | d |
|---|---|---|---|---|
| Surlyn 8945 | 55 | 45 | 27 | 20 |
| Himilan AM7329 | 45 | 45 | 45 | 25 |
| Rabalon T3221C | - | 10 | 28 | 55 |
| Titanium dioxide | 3 | 3 | 3 | 3 |
| Hardness (Shore D) | 65 | 56 | 48 | 29 |

**Table I-5 Composition and Hardness of Cover (parts by weight)**

| Type | A | B | C | D |
|---|---|---|---|---|
| Elastollan NY82A | 100 | - | - | - |
| Elastollan NY85A | - | 50 | - | - |
| Elastollan NY90A | - | 50 | - | - |
| Elastollan NY97A | - | - | 100 | - |
| Surlyn 8945 | - | - | - | 40 |
| Himilan AM7329 | - | - | - | 55 |
| Rabalon T3221C | - | - | - | 5 |
| TINUVIN 770 | 0.2 | 0.2 | 0.2 | 0.2 |
| Titanium dioxide | 4 | 4 | 4 | 4 |
| Ultramarine blue | 0.04 | 0.04 | 0.04 | 0.04 |
| Hardness Hc (Shore D) | 29 | 36 | 47 | 60 |

**Table I-6 Results of Evaluation**

| | Ex.I-1 | Ex.I-2 | Ex.I-3 | Ex.I-4 | Ex.I-5 |
|---|---|---|---|---|---|
| Core Type | (3) | (4) | (5) | (6) | (7) |
| Diameter (mm) | 38.5 | 38.5 | 38.5 | 38.5 | 38.5 |
| Hs - H(0.0) | 31.5 | 32.5 | 31.5 | 27.5 | 13.0 |
| R² | 0.96 | 0.99 | 0.99 | 0.99 | 0.95 |
| Gradient | 0.28 | 0.33 | 0.32 | 0.26 | 0.11 |

| Inner mid layer | | | | | |
|---|---|---|---|---|---|
| Type | a | a | a | a | a |
| Hm1 (Shore D) | 65 | 65 | 65 | 65 | 65 |
| Diameter (mm) | 40.1 | 40.1 | 40.1 | 40.1 | 40.1 |
| T1 (mm) | 0.8 | 0.8 | 0.8 | 0.8 | 0.8 |

| Outer mid layer | | | | | |
|---|---|---|---|---|---|
| Type | c | c | c | c | c |
| Hm2 (Shore D) | 48 | 48 | 48 | 48 | 48 |
| Diameter (mm) | 41.7 | 41.7 | 41.7 | 41.7 | 41.7 |
| T2 (mm) | 0.8 | 0.8 | 0.8 | 0.8 | 0.8 |
| Cover Type | A | A | A | A | A |
| Hc (Shore D) | 29 | 29 | 29 | 29 | 29 |
| Tc (mm) | 0.5 | 0.5 | 0.5 | 0.5 | 0.5 |
| Hm1 - Hm2 | 17 | 17 | 17 | 17 | 17 |
| Hm1 - Hc | 36 | 36 | 36 | 36 | 36 |
| T1 + T2 (mm) | 1.6 | 1.6 | 1.6 | 1.6 | 1.6 |

| Ball | | | | | |
|---|---|---|---|---|---|
| Db (mm) | 2.6 | 2.6 | 2.6 | 2.6 | 2.6 |
| (W#1) spin (rpm) | 3200 | 3100 | 3150 | 3200 | 3280 |
| (W#1) flight (m) | 239 | 241 | 240 | 239 | 235 |
| (SW) spin (rpm) | 6850 | 6800 | 6800 | 6800 | 6850 |
| Durability | 110 | 115 | 113 | 110 | 103 |
| Feel at impact | A | A | A | A | B |

**Table I-7 Results of Evaluation**

| | Ex.I-6 | Ex.I-7 | Ex.I-8 | Ex.I-9 | Ex.I-10 |
|---|---|---|---|---|---|
| Core Type | (8) | (9) | (10) | (11) | (12) |
| Diameter (mm) | 38.5 | 38.5 | 38.5 | 38.5 | 38.5 |
| Hs - H(0.0) | 31.5 | 30.0 | 32.0 | 31.5 | 32.5 |
| R² | 0.97 | 0.98 | 0.97 | 0.98 | 0.99 |
| Gradient | 0.31 | 0.31 | 0.32 | 0.32 | 0.32 |

| Inner mid layer | | | | | |
|---|---|---|---|---|---|
| Type | a | a | a | a | a |
| Hm1 (Shore D) | 65 | 65 | 65 | 65 | 65 |
| Diameter (mm) | 40.1 | 40.1 | 40.1 | 40.1 | 40.1 |
| T1 (mm) | 0.8 | 0.8 | 0.8 | 0.8 | 0.8 |

| Outer mid layer | | | | | |
|---|---|---|---|---|---|
| Type | c | c | c | c | c |
| Hm2 (Shore D) | 48 | 48 | 48 | 48 | 48 |
| Diameter (mm) | 41.7 | 41.7 | 41.7 | 41.7 | 41.7 |
| T2 (mm) | 0.8 | 0.8 | 0.8 | 0.8 | 0.8 |
| Cover Type | A | A | A | A | A |
| Hc (Shore D) | 29 | 29 | 29 | 29 | 29 |
| Tc (mm) | 0.5 | 0.5 | 0.5 | 0.5 | 0.5 |
| Hm1 - Hm2 | 17 | 17 | 17 | 17 | 17 |
| Hm1 - Hc | 36 | 36 | 36 | 36 | 36 |
| T1 + T2 (mm) | 1.6 | 1.6 | 1.6 | 1.6 | 1.6 |

| Ball | | | | | |
|---|---|---|---|---|---|
| Db (mm) | 2.6 | 2.6 | 2.6 | 2.6 | 2.6 |
| (W#1) spin (rpm) | 3200 | 3150 | 3200 | 3150 | 3150 |
| (W#1) flight (m) | 239 | 240 | 238 | 239 | 240 |
| (SW) spin (rpm) | 6850 | 6800 | 6850 | 6800 | 6800 |
| Durability | 110 | 113 | 110 | 113 | 112 |
| Feel at impact | A | A | A | A | A |

**Table I-8 Results of Evaluation**

| | Ex.I-11 | Ex.I-12 | Ex.I-13 | Ex.I-14 | Ex.I-15 |
|---|---|---|---|---|---|
| Core Type | (13) | (4) | (4) | (4) | (15) |
| Diameter (mm) | 38.5 | 38.5 | 38.5 | 37.7 | 35.3 |
| Hs - H(0.0) | 32.5 | 32.5 | 32.5 | 32.5 | 32.5 |
| R² | 0.99 | 0.99 | 0.99 | 0.99 | 0.99 |
| Gradient | 0.33 | 0.33 | 0.33 | 0.33 | 0.33 |

| Inner mid layer | | | | | |
|---|---|---|---|---|---|
| Type | a | a | a | a | a |
| Hm1 (Shore D) | 65 | 65 | 65 | 65 | 65 |
| Diameter (mm) | 40.1 | 40.1 | 40.1 | 39.3 | 38.5 |
| T1 (mm) | 0.8 | 0.8 | 0.8 | 0.8 | 1.6 |

| Outer mid layer | | | | | |
|---|---|---|---|---|---|
| Type | c | c | c | c | c |
| Hm2 (Shore D) | 48 | 48 | 48 | 48 | 48 |
| Diameter (mm) | 41.7 | 41.7 | 41.7 | 40.9 | 41.7 |
| T2 (mm) | 0.8 | 0.8 | 0.8 | 0.8 | 1.6 |

| Cover Type | A | B | C | A | A |
|---|---|---|---|---|---|
| Hc (Shore D) | 29 | 36 | 47 | 29 | 29 |
| Tc (mm) | 0.5 | 0.5 | 0.5 | 0.9 | 0.5 |
| Hm1 - Hm2 | 17 | 17 | 17 | 17 | 17 |
| Hm1 - Hc | 36 | 29 | 18 | 36 | 36 |
| T1 + T2 (mm) | 1.6 | 1.6 | 1.6 | 1.6 | 3.2 |

| Ball | | | | | |
|---|---|---|---|---|---|
| Db (mm) | 2.6 | 2.6 | 2.6 | 2.6 | 2.5 |
| (W#1) spin (rpm) | 3100 | 3000 | 2950 | 3250 | 3150 |
| (W#1) flight (m) | 241 | 244 | 245 | 237 | 239 |
| (SW) spin (rpm) | 6800 | 6650 | 6500 | 7000 | 6900 |
| Durability | 115 | 112 | 107 | 115 | 116 |
| Feel at impact | A | A | B | A | B |

**Table I-9 Results of Evaluation**

| | Ex.I-16 | Ex.I-17 |
|---|---|---|
| Core Type | (4) | (14) |
| Diameter (mm) | 38.5 | 38.5 |
| Hs - H(0.0) | 32.5 | 32.5 |
| R² | 0.99 | 0.99 |
| Gradient | 0.33 | 0.33 |

| Inner mid layer | | |
|---|---|---|
| Type | a | a |
| Hm1 (Shore D) | 65 | 65 |
| Diameter (mm) | 40.1 | 40.1 |
| T1 (mm) | 0.8 | 0.8 |

| Outer mid layer | | |
|---|---|---|
| Type | b | d |
| Hm2 (Shore D) | 56 | 29 |
| Diameter (mm) | 41.7 | 41.7 |
| T2 (mm) | 0.8 | 0.8 |

| Cover Type | A | A |
|---|---|---|
| Hc (Shore D) | 29 | 29 |
| Tc (mm) | 0.5 | 0.5 |
| Hm1 - Hm2 | 9 | 36 |
| Hm1 - Hc | 36 | 36 |
| T1 + T2 (mm) | 1.6 | 1.6 |
| Ball | | |
| Db (mm) | 2.6 | 2.6 |
| (W#1) spin (rpm) | 3050 | 3200 |
| (W#1) flight (m) | 242 | 238 |
| (SW) spin (rpm) | 6650 | 6850 |
| Durability | 112 | 117 |
| Feel at impact | B | A |

**Table I-10 Results of Evaluation**

| | Comp. Ex.I-1 | Comp. Ex.I-2 | Comp. Ex.I-3 | Comp. Ex.I-4 | Comp. Ex. I-5 | Comp. Ex.I-6 |
|---|---|---|---|---|---|---|
| Core Type | (1) | (4) | (15) | (15) | (14) | (2) |
| Diameter (mm) | 38.5 | 38.5 | 38.5 | 38.5 | 38.5 | 38.5 |
| Hs - H(0.0) | 30.0 | 32.5 | 32.5 | 32.5 | 32.5 | 31.0 |
| R² | 0.86 | 0.99 | 0.99 | 0.99 | 0.99 | 0.90 |
| Gradient | 0.23 | 0.33 | 0.33 | 0.33 | 0.33 | 0.25 |

| Inner mid layer | | | | | | |
|---|---|---|---|---|---|---|
| Type | a | c | b | a | c | a |
| Hm1 (Shore D) | 65 | 48 | 56 | 65 | 48 | 65 |
| Diameter (mm) | 40.1 | 40.1 | 40.1 | 40.1 | 40.1 | 40.1 |
| T1 (mm) | 0.8 | 0.8 | 0.8 | 0.8 | 0.8 | 0.8 |

| Outer mid layer | | | | | | |
|---|---|---|---|---|---|---|
| Type | c | a | c | a | c | c |
| Hm2 (Shore D) | 48 | 65 | 48 | 65 | 48 | 48 |
| Diameter (mm) | 41.7 | 41.7 | 41.7 | 41.7 | 41.7 | 41.7 |
| T2 (mm) | 0.8 | 0.8 | 0.8 | 0.8 | 0.8 | 0.8 |

| Cover Type | A | A | D | A | A | A |
|---|---|---|---|---|---|---|
| Hc (Shore D) | 29 | 29 | 60 | 29 | 29 | 29 |
| Tc (mm) | 0.5 | 0.5 | 0.5 | 0.5 | 0.5 | 0.5 |
| Hm1 - Hm2 | 17 | -17 | 8 | 0 | 0 | 17 |
| Hm1 - Hc | 36 | 19 | -4 | 36 | 19 | 36 |
| T1 + T2 (mm) | 1.6 | 1.6 | 1.6 | 1.6 | 1.6 | 1.6 |

| Ball | | | | | | |
|---|---|---|---|---|---|---|
| Db (mm) | 2.6 | 2.6 | 2.6 | 2.6 | 2.6 | 2.6 |
| (W#1) spin (rpm) | 3350 | 3000 | 2850 | 2900 | 3300 | 3300 |
| (W#1) flight (m) | 233 | 244 | 247 | 246 | 234 | 234 |
| (SW) spin (rpm) | 6850 | 6700 | 5800 | 6400 | 6900 | 6850 |
| Durability | 100 | 80 | 102 | 75 | 130 | 103 |
| Feel at impact | B | C | C | D | B | B |

As shown in Tables I-6 to I-10, the golf balls according to Examples are excellent in various performance characteristics. From the results of evaluation, advantages of the present invention are clear.

### [Experiment 2]

### [Example II-1]

A rubber composition was obtained by kneading 100 parts by weight of a high-cis polybutadiene (trade name "BR-730", manufactured by JSR Corporation), 38 parts by weight of zinc diacrylate (trade name "Sanceler SR", manufactured by SANSHIN CHEMICAL INDUSTRY CO., LTD.), 5 parts by weight of zinc oxide, an appropriate amount of barium sulfate, 0.2 parts by weight of 2-thionaphthol, 0.9 parts by weight of dicumyl peroxide (trade name "PercumylD" manufactured by NOF Corporation), and 2.0 parts by weight of zinc octoate (a product of Mitsuwa Chemicals Co. , Ltd.). This rubber composition was placed into a mold including upper and lower mold halves each having a hemispherical cavity, and heated at 170°C for 25 minutes to obtain a spherical core with a diameter of 38.5 mm. The amount of barium sulfate was adjusted such that the weight of a golf ball is 45.6 g.

A resin composition was obtained by kneading 25 parts by weight of an ionomer resin (the aforementioned "Surlyn 8945"), 45 parts by weight of another ionomer resin (the aforementioned "Himilan AM7329"), 30 parts by weight of a styrene block-containing thermoplastic elastomer (the aforementioned "Rabalon T3221C"), and 3 parts by weight of titanium dioxide with a twin-screw kneading extruder. The extruding conditions were a screw diameter of 45 mm, a screw rotational speed of 200 rpm, screw L/D of 35, and a die temperature of 160 to 230°C. The core was placed into a mold. The resin composition was injected around the core by injection molding to form an inner mid layer with a thickness of 0.8 mm.

A resin composition was obtained by kneading 55 parts by weight of an ionomer resin (the aforementioned "Surlyn 8945"), 45 parts by weight of another ionomer resin (the aforementioned "Himilan AM7329"), and 3 parts by weight of titanium dioxide with a twin-screw kneading extruder under the above extruding conditions. The sphere consisting of the core and the inner mid layer was placed into a mold. The resin composition was injected around the sphere by injection molding to form an outer mid layer with a thickness of 0.8 mm.

A paint composition (trade name "POLIN 750LE", manufactured by SHINTO PAINT CO., LTD.) including a two-component curing type epoxy resin as a base polymer was prepared. The base material liquid of this paint composition includes 30 parts by weight of a bisphenol A type solid epoxy resin and 70 parts by weight of a solvent. The curing agent liquid of this paint composition includes 40 parts by weight of a modified polyamide amine, 55 parts by weight of a solvent, and 5 parts by weight of titanium dioxide. The weight ratio of the base material liquid to the curing agent liquid is 1/1. This paint composition was applied to the surface of the outer mid layer with an air gun, and kept at 23°C for 12 hours to obtain a reinforcing layer with a thickness of 6 µm.

A resin composition was obtained by kneading 100 parts by weight of a thermoplastic polyurethane elastomer (the aforementioned "Elastollan NY82A"), 0.2 parts by weight of a hindered amine light stabilizer (trade name "TINUVIN 770", manufactured by Ciba Japan K.K.) , 4 parts by weight of titanium dioxide, and 0.04 parts by weight of ultramarine blue with a twin-screw kneading extruder under the above extruding conditions. Half shells were formed from this resin composition by compression molding. The sphere consisting of the core, the inner mid layer, the outer mid layer, and the reinforcing layer was covered with two of these half shells. The sphere and the half shells were placed into a final mold that includes upper and lower mold halves each having a hemispherical cavity and that has a large number of pimples on its cavity face. A cover was obtained by compression molding. The thickness of the cover was 0.5 mm. Dimples having a shape that is the inverted shape of the pimples were formed on the cover. The surface of the cover was polished. A clear paint including a two-component curing type polyurethane as a base material was applied to this cover with an air gun and was dried and cured to obtain a golf ball of Example II-1 with a diameter of 42.7 mm and a weight of 45.6 g.

### [Examples II-2 to 11-16 and Comparative Examples II-1 to II-7]

Golf balls of Examples II-2 to 11-16 and Comparative Examples II-1 to II-7 were obtained in the same manner as Example II-1, except the specifications of the core, the inner mid layer, the outer mid layer, and the cover were as shown in Tables II-6 to II-11 below. The composition and hardness of the core are shown in detail in Tables II-1 to II-3 below. The compositions and hardnesses of the inner mid layer and the outer mid layer are shown in Table II-4 below. The composition and hardness of the cover are shown in Table II-5 below.

### [Hit with Driver (W#1)]

A driver with a titanium head (trade name "XXIO", manufactured by DUNLOP SPORTS CO. LTD., shaft hardness: S, loft angle: 10.0°) was attached to a swing machine manufactured by True Temper Co. A golf ball was hit under the condition of a head speed of 45 m/sec. The spin rate was measured immediately after the hit. Furthermore, the flight distance from the launch point to the stop point was measured. The average value of data obtained by 10 measurements is shown in Tables II-6 to II-11 below.

### [Hit with Sand Wedge (SW)]

A sand wedge (trade name "XXIO", manufactured by DUNLOP SPORTS CO. LTD., shaft hardness: R, loft angle: 56.0°) was attached to a swing machine manufactured by True Temper Co. A golf ball was hit under the condition of a head speed of 21 m/sec. The backspin rate was measured immediately after the hit. The average value of data obtained by 10 measurements is shown in Tables II-6 to II-11 below.

### [Durability]

A driver with a titanium head (trade name "XXIO", manufactured by DUNLOP SPORTS CO. LTD., shaft hardness: S, loft angle: 10.0°) was attached to a swing robot M/C manufactured by True Temper Co. A golf ball having been kept at 23°C for 12 hours was used for the measurement. The golf ball was repeatedly hit under the condition of a head speed of 45 m/sec. The number of hits required to break the golf ball was measured. An index of the average value of data obtained for 12 golf balls is shown in Tables II-6 to II-11 below. The higher the index is, the more excellent the durability of the golf ball is.

**Table II-1 Composition and Hardness of Core (parts by weight)**

| Type | (1) | (2) | (3) | (4) | (5) |
|---|---|---|---|---|---|
| BR-730 | 100 | 100 | 100 | 100 | 100 |
| Sanceler SR | 34 | 38 | 38 | 38 | 39 |
| ZN-DA90S | - | - | - | - | - |
| Zinc oxide | 5 | 5 | 5 | 5 | 5 |
| Barium sulfate | * | * | * | * | * |
| 2-thionaphthol | 0.2 | 0.2 | 0.2 | 0.2 | 0.2 |
| Bis(pentabromophenyl ) disulfide | - | - | - | - | - |
| Dicumyl peroxide | 0.9 | 0.9 | 0.9 | 0.9 | 0.9 |
| Zinc octoate | - | 0.5 | 2 | 5 | 10 |
| Zinc stearate | - | - | - | - | - |
| Zinc myristate | - | - | - | - | - |
| Amount of acid/salt | 0 | 0.5 | 2 | 5 | 10 |
| Vulc. conditions | | | | | |
| Temperature (°C) | 170 | 170 | 170 | 170 | 170 |
| Time (min) | 25 | 25 | 25 | 25 | 25 |

| Hardness distribution (JIS-C hardness) | | | | | |
|---|---|---|---|---|---|
| H(0.0) | 57.0 | 55.0 | 55.0 | 56.5 | 55.5 |
| H(12.5) | 68.0 | 65.5 | 62.0 | 59.5 | 59.0 |
| H(25.0) | 73.0 | 70.5 | 67.5 | 64.5 | 64.0 |
| H(37.5) | 74.0 | 72.0 | 69.5 | 67.0 | 67.0 |
| H(50.0) | 74.0 | 73.5 | 71.5 | 70.0 | 69.5 |
| H(62.5) | 74.0 | 75.0 | 72.5 | 74.0 | 72.0 |
| H(75.0) | 78.0 | 76.5 | 77.5 | 80.5 | 80.0 |
| H(87.5) | 82.0 | 81.5 | 82.5 | 85.0 | 84.0 |
| Surface hardness Hs | 87.0 | 86.0 | 86.5 | 89.0 | 87.0 |

| | | | | | |
|---|---|---|---|---|---|
| * Appropriate amount | | | | | |

**Table II-2 Composition and Hardness of Core (parts by weight)**

| Type | (6) | (7) | (8) | (9) | (10) |
|---|---|---|---|---|---|
| BR-730 | 100 | 100 | 100 | 100 | 100 |
| Sanceler SR | 40 | 41 | 35 | 36 | 38 |
| ZN-DA90S | - | - | - | - | - |
| Zinc oxide | 5 | 5 | 5 | 5 | 5 |
| Barium sulfate | * | * | * | * | * |
| 2-thionaphthol | 0.2 | 0.2 | 0.2 | 0.2 | 0.2 |
| Bis(pentabromophenyl ) disulfide | - | - | - | - | - |
| Dicumyl peroxide | 0.9 | 0.9 | 0.9 | 0.9 | 0.9 |
| Zinc octoate | 30 | 45 | - | - | - |
| Zinc stearate | - | - | 10 | 20 | - |
| Zinc myristate | - | - | - | - | 5 |
| Amount of acid/salt | 30 | 45 | 10 | 20 | 5 |

| Vulc.conditions | | | | | |
|---|---|---|---|---|---|
| Temperature (°C) | 170 | 170 | 170 | 170 | 170 |
| Time (min) | 25 | 25 | 25 | 25 | 25 |

| Hardness distribution (JIS-C hardness) | | | | | |
|---|---|---|---|---|---|
| H(0.0) | 53.5 | 64.0 | 57.5 | 56.0 | 57.0 |
| H(12.5) | 58.5 | 68.0 | 61.0 | 59.0 | 60.5 |
| H(25.0) | 61.5 | 69.5 | 65.5 | 62.0 | 65.0 |
| H(37.5) | 65.0 | 71.0 | 68.0 | 65.5 | 68.0 |
| H(50.0) | 68.0 | 71.5 | 70.0 | 69.0 | 70.0 |
| H(62.5) | 70.5 | 72.5 | 71.5 | 71.0 | 72.0 |
| H(75.0) | 73.5 | 73.5 | 81.0 | 80.0 | 80.5 |
| H(87.5) | 76.0 | 76.0 | 85.0 | 82.0 | 85.0 |
| Surface hardness Hs | 81.0 | 77.0 | 89.0 | 86.0 | 89.0 |

| | | | | | |
|---|---|---|---|---|---|
| * Appropriate amount | | | | | |

**Table II-3 Composition and Hardness of Core (parts by weight)**

| Type | (11) | (12) | (13) | (14) | (15) |
|---|---|---|---|---|---|
| BR-730 | 100 | 100 | 100 | 100 | 100 |
| Sanceler SR | 39 | 40 | - | 39 | 37 |
| ZN-DA90S | - | - | 38 | - | - |
| Zinc oxide | 5 | 5 | 5 | 5 | 5 |
| Barium sulfate | * | * | * | * | * |
| 2-thionaphthol | 0.2 | - | 0.2 | 0.2 | 0.2 |
| Bis(pentabromophenyl ) disulfide | - | 0.3 | - | - | - |
| Dicumyl peroxide | 0.9 | 0.9 | 0.9 | 0.9 | 0.9 |
| Zinc octoate | - | 5 | 5 | 5 | 5 |
| Zinc stearate | - | - | - | - | - |
| Zinc myristate | 10 | - | - | - | - |
| Amount of acid/salt | 10 | 5 | 5 | 5 | 5 |
| Vulc. conditions | | | | | |
| Temperature (°C) | 170 | 170 | 170 | 170 | 170 |
| Time (min) | 25 | 25 | 25 | 25 | 25 |

| Hardness distribution (JIS-C hardness) | | | | | |
|---|---|---|---|---|---|
| H(0.0) | 56.0 | 56.5 | 56.5 | 57.0 | 56.0 |
| H(12.5) | 59.5 | 59.5 | 59.5 | 60.0 | 59.0 |
| H(25.0) | 64.5 | 65.0 | 64.5 | 65.0 | 64.0 |
| H(37.5) | 67.5 | 67.0 | 67.0 | 67.5 | 66.5 |
| H(50.0) | 69.5 | 70.0 | 71.0 | 70.5 | 69.5 |
| H(62.5) | 72.0 | 74.0 | 74.0 | 74.5 | 73.5 |
| H(75.0) | 80.5 | 80.0 | 80.5 | 81.0 | 80.0 |
| H(87.5) | 84.5 | 85.0 | 85.0 | 85.5 | 84.5 |
| Surface hardness Hs | 87.5 | 89.0 | 89.0 | 89.5 | 88.5 |

| | | | | | |
|---|---|---|---|---|---|
| * Appropriate amount | | | | | |

The details of the compounds listed in Tables II-1 to II-3 are as follows.
BR730: a high-cis polybutadiene manufactured by JSR Corporation (cis-1, 4-bond content: 96% by weight, 1, 2-vinyl bond content: 1.3% by weight, Mooney viscosity (ML₁₊₄ (100°C)): 55, molecular weight distribution (Mw/Mn): 3)
Sanceler SR: zinc diacrylate manufactured by SANSHIN CHEMICAL INDUSTRY CO., LTD. (a product coated with 10% by weight of stearic acid)
ZN-DA90S: zinc diacrylate manufactured by Nihon Jyoryu Kogyo Co., Ltd. (a product coated with 10% by weight of zinc stearate)
Zinc oxide: trade name "Ginrei R" manufactured by Toho Zinc Co., Ltd.
Barium sulfate: trade name "Barium Sulfate BD" manufactured by Sakai Chemical Industry Co., Ltd.
2-thionaphthol: a product of Tokyo Chemical Industry Co. , Ltd.
Bis(pentabromophenyl)disulfide: a product of Kawaguchi Chemical Industry Co., LTD.
Dicumyl peroxide: trade name "Percumyl D" manufactured by NOF Corporation
Zinc octoate: a product of Mitsuwa Chemicals Co., Ltd. (purity: 99% or greater)
Zinc stearate: a product of Wako Pure Chemical Industries, Ltd. (purity: 99% or greater)
Zinc myristate: a product of NOF Corporation (purity: 90% or greater)

**Table II-4 Compositions and Hardnesses of Inner Mid Layer and Outer Mid Layer (parts by weight)**

| Type | a | b | c | d |
|---|---|---|---|---|
| Surlyn 8945 | 55 | 45 | 25 | 20 |
| Himilan AM7329 | 45 | 45 | 45 | 25 |
| Rabalon T3221C | - | 10 | 30 | 55 |
| Titanium dioxide | 3 | 3 | 3 | 3 |
| Hardness (Shore D) | 65 | 56 | 47 | 29 |

**Table II-5 Composition and Hardness of Cover (parts by weight)**

| Type | A | B | C | D |
|---|---|---|---|---|
| Elastollan NY82A | 100 | - | - | - |
| Elastollan NY85A | - | 50 | - | - |
| Elastollan NY90A | - | 50 | - | - |
| Elastollan NY97A | - | - | 100 | - |
| Surlyn 8945 | - | - | - | 40 |
| Himilan AM7329 | - | - | - | 55 |
| Rabalon T3221C | - | - | - | 5 |
| TINUVIN 770 | 0.2 | 0.2 | 0.2 | 0.2 |
| Titanium dioxide | 4 | 4 | 4 | 4 |
| Ultramarine blue | 0.04 | 0.04 | 0.04 | 0.04 |
| Hardness Hc (Shore D) | 29 | 36 | 47 | 60 |

**Table II-6 Results of Evaluation**

| | Ex. II-1 | Ex. II-2 | Ex. II-3 | Ex. II-4 |
|---|---|---|---|---|
| Core | | | | |
| Type | (3) | (4) | (5) | (6) |
| Diameter (mm) | 38.5 | 38.5 | 38.5 | 38.5 |
| Hs - H(0.0) | 31.5 | 32.5 | 31.5 | 27.5 |
| R² | 0.96 | 0.99 | 0.99 | 0.99 |
| Gradient | 0.28 | 0.33 | 0.32 | 0.26 |

| Inner mid layer | | | | |
|---|---|---|---|---|
| Type | c | c | c | c |
| Hm1 (Shore D) | 47 | 47 | 47 | 47 |
| Diameter (mm) | 40.1 | 40.1 | 40.1 | 40.1 |
| T1 (mm) | 0.8 | 0.8 | 0.8 | 0.8 |

| Outer mid layer | | | | |
|---|---|---|---|---|
| Type | a | a | a | a |
| Hm2 (Shore D) | 65 | 65 | 65 | 65 |
| Diameter (mm) | 41.7 | 41.7 | 41.7 | 41.7 |
| T2 (mm) | 0.8 | 0.8 | 0.8 | 0.8 |
| Cover Type | A | A | A | A |
| Hc (Shore D) | 29 | 29 | 29 | 29 |
| Tc (mm) | 0.5 | 0.5 | 0.5 | 0.5 |
| Hm2 - Hm1 | 18 | 18 | 18 | 18 |
| Hm2 - Hc | 36 | 36 | 36 | 36 |
| T1 + T2 (mm) | 1.6 | 1.6 | 1.6 | 1.6 |

| Ball | | | | |
|---|---|---|---|---|
| Db (mm) | 2.6 | 2.6 | 2.6 | 2.6 |
| (W#1) spin (rpm) | 3100 | 3000 | 3050 | 3100 |
| (W#1) flight (m) | 241 | 244 | 243 | 241 |
| (SW) spin (rpm) | 6750 | 6700 | 6700 | 6700 |
| Durability | 107 | 110 | 109 | 108 |

**Table II-7 Results of Evaluation**

| | Ex. II-5 | Ex. 11-6 | Ex.II-7 | Ex.II-8 |
|---|---|---|---|---|
| Core | | | | |
| Type | (7) | (8) | (9) | (10) |
| Diameter (mm) | 38.5 | 38.5 | 38.5 | 38.5 |
| Hs - H(0.0) | 13.0 | 31.5 | 30.0 | 32.0 |
| R² | 0.95 | 0.97 | 0.98 | 0.97 |
| Gradient | 0.11 | 0.31 | 0.31 | 0.32 |

| Inner mid layer | | | | |
|---|---|---|---|---|
| Type | c | c | c | c |
| Hm1 (Shore D) | 47 | 47 | 47 | 47 |
| Diameter (mm) | 40.1 | 40.1 | 40.1 | 40.1 |
| T1 (mm) | 0.8 | 0.8 | 0.8 | 0.8 |

| Outer mid layer | | | | |
|---|---|---|---|---|
| Type | a | a | a | a |
| Hm2 (Shore D) | 65 | 65 | 65 | 65 |
| Diameter (mm) | 41.7 | 41.7 | 41.7 | 41.7 |
| T2 (mm) | 0.8 | 0.8 | 0.8 | 0.8 |
| Cover Type | A | A | A | A |
| Hc (Shore D) | 29 | 29 | 29 | 29 |
| Tc (mm) | 0.5 | 0.5 | 0.5 | 0.5 |
| Hm2 - Hm1 | 18 | 18 | 18 | 18 |
| Hm2 - Hc | 36 | 36 | 36 | 36 |
| T1 + T2 (mm) | 1.6 | 1.6 | 1.6 | 1.6 |

| Ball | | | | |
|---|---|---|---|---|
| Db (mm) | 2.6 | 2.6 | 2.6 | 2.6 |
| (W#1) spin (rpm) | 3300 | 3100 | 3050 | 3100 |
| (W#1) flight(m) | 234 | 241 | 243 | 240 |
| (SW) spin (rpm) | 6750 | 6750 | 6700 | 6750 |
| Durability | 104 | 107 | 109 | 107 |

**Table II-8 Results of Evaluation**

| | Ex.II-9 | Ex. II-10 | Ex. II-11 | Ex. II-12 |
|---|---|---|---|---|
| Core | | | | |
| Type | (11) | (12) | (13) | (14) |
| Diameter (mm) | 38.5 | 38.5 | 38.5 | 38.5 |
| Hs - H(0.0) | 31.5 | 32.5 | 32.5 | 32.5 |
| R² | 0.98 | 0.99 | 0.99 | 0.99 |
| Gradient | 0.32 | 0.32 | 0.33 | 0.33 |

| Inner mid layer | | | | |
|---|---|---|---|---|
| Type | c | c | c | c |
| Hm1 (Shore D) | 47 | 47 | 47 | 47 |
| Diameter (mm) | 40.1 | 40.1 | 40.1 | 40.1 |
| T1 (mm) | 0.8 | 0.8 | 0.8 | 0.8 |

| Outer mid layer | | | | |
|---|---|---|---|---|
| Type | a | a | a | a |
| Hm2 (Shore D) | 65 | 65 | 65 | 65 |
| Diameter (mm) | 41.7 | 41.7 | 41.7 | 41.7 |
| T2 (mm) | 0.8 | 0.8 | 0.8 | 0.8 |
| Cover Type | A | A | A | B |
| Hc (Shore D) | 29 | 29 | 29 | 36 |
| Tc (mm) | 0.5 | 0.5 | 0.5 | 0.5 |
| Hm2 - Hm1 | 18 | 18 | 18 | 18 |
| Hm2 - Hc | 36 | 36 | 36 | 29 |
| T1 + T2 (mm) | 1.6 | 1.6 | 1.6 | 1.6 |

| Ball | | | | |
|---|---|---|---|---|
| Db (mm) | 2.6 | 2.6 | 2.6 | 2.6 |
| (W#1) spin (rpm) | 3050 | 3050 | 3000 | 2900 |
| (W#1) flight (m) | 242 | 243 | 244 | 246 |
| (SW) spin (rpm) | 6700 | 6700 | 6700 | 6550 |
| Durability | 109 | 108 | 110 | 108 |

**Table II-9 Results of Evaluation**

| | EX. II-13 | Ex. II-14 | Ex. II-15 | Ex. II-16 |
|---|---|---|---|---|
| Core | | | | |
| Type | (4) | (4) | (15) | (14) |
| Diameter (mm) | 38.5 | 37.7 | 35.3 | 38.5 |
| Hs - H(0.0) | 32.5 | 32.5 | 32.5 | 32.5 |
| R² | 0.99 | 0.99 | 0.99 | 0.99 |
| Gradient | 0.33 | 0.33 | 0.33 | 0.33 |

| Inner mid layer | | | | |
|---|---|---|---|---|
| Type | c | c | c | d |
| Hm1 (Shore D) | 47 | 47 | 47 | 29 |
| Diameter (mm) | 40.1 | 39.3 | 38.5 | 40.1 |
| T1 (mm) | 0.8 | 0.8 | 1.6 | 0.8 |

| Outer mid layer | | | | |
|---|---|---|---|---|
| Type | a | a | a | a |
| Hm2 (Shore D) | 65 | 65 | 65 | 65 |
| Diameter (mm) | 41.7 | 40.9 | 41.7 | 41.7 |
| T2 (mm) | 0.8 | 0.8 | 1.6 | 0.8 |
| Cover Type | C | A | A | A |
| Hc (Shore D) | 47 | 29 | 29 | 29 |
| Tc (mm) | 0.5 | 0.9 | 0.5 | 0.5 |
| Hm2 - Hml | 18 | 18 | 18 | 36 |
| Hm2 - Hc | 18 | 36 | 36 | 36 |
| T1 + T2 (mm) | 1.6 | 1.6 | 3.2 | 1.6 |

| Ball | | | | |
|---|---|---|---|---|
| Db (mm) | 2.6 | 2.6 | 2.5 | 2.6 |
| (W#1) spin (rpm) | 2850 | 3150 | 3050 | 3100 |
| (W#1) flight (m) | 247 | 240 | 240 | 239 |
| (SW) spin (rpm) | 6400 | 6900 | 6600 | 6750 |
| Durability | 106 | 110 | 112 | 112 |

**Table II-10 Results of Evaluation**

| | Comp. Ex. II-1 | Comp. Ex. II-2 | Comp. Ex. II-3 | Comp. Ex. II-4 |
|---|---|---|---|---|
| Core | | | | |
| Type | (1) | (2) | (4) | (4) |
| Diameter (mm) | 38.5 | 38.5 | 38.5 | 38.5 |
| Hs - H(0.0) | 30.0 | 31.0 | 32.5 | 32.5 |
| R² | 0.86 | 0.90 | 0.99 | 0.99 |
| Gradient | 0.23 | 0.25 | 0.33 | 0.33 |

| Inner mid layer | | | | |
|---|---|---|---|---|
| Type | c | c | b | a |
| Hm1 (Shore D) | 47 | 47 | 56 | 65 |
| Diameter (mm) | 40.1 | 40.1 | 40.1 | 40.1 |
| T1 (mm) | 0.8 | 0.8 | 0.8 | 0.8 |

| Outer mid layer | | | | |
|---|---|---|---|---|
| Type | a | a | a | c |
| Hm2 (Shore D) | 65 | 65 | 65 | 47 |
| Diameter (mm) | 41.7 | 41.7 | 41.7 | 41.7 |
| T2 (mm) | 0.8 | 0.8 | 0.8 | 0.8 |
| Cover Type | A | A | A | A |
| Hc (Shore D) | 29 | 29 | 29 | 29 |
| Tc (mm) | 0.5 | 0.5 | 0.5 | 0.5 |
| Hm2 - Hm1 | 18 | 18 | 9 | -18 |
| Hm2 - Hc | 36 | 36 | 36 | 18 |
| T1 + T2 (mm) | 1.6 | 1.6 | 1.6 | 1.6 |

| Ball | | | | |
|---|---|---|---|---|
| Db (mm) | 2.6 | 2.6 | 2.5 | 2.6 |
| (W#1) spin (rpm) | 3250 | 3200 | 2950 | 3100 |
| (W#1) flight (m) | 235 | 237 | 245 | 241 |
| (SW) spin (rpm) | 6750 | 6750 | 6550 | 6800 |
| Durability | 100 | 103 | 109 | 120 |

**Table II-11 Results of Evaluation**

| | Comp. Ex. II-5 | Comp. Ex.II-6 | Comp. Ex.II-7 |
|---|---|---|---|
| Core | | | |
| Type | (15) | (15) | (14) |
| Diameter (mm) | 38.5 | 38.5 | 38.5 |
| Hs - H(0.0) | 32.5 | 32.5 | 32.5 |
| R² | 0.99 | 0.99 | 0.99 |
| Gradient | 0.33 | 0.33 | 0.33 |

| Inner mid layer | | | |
|---|---|---|---|
| Type | c | a | c |
| Hm1 (Shore D) | 47 | 65 | 47 |
| Diameter (mm) | 40.1 | 40.1 | 40.1 |
| T1 (mm) | 0.8 | 0.8 | 0.8 |

| Outer mid layer | | | |
|---|---|---|---|
| Type | b | a | c |
| Hm2 (Shore D) | 56 | 65 | 47 |
| Diameter (mm) | 41.7 | 41.7 | 41.7 |
| T2 (mm) | 0.8 | 0.8 | 0.8 |
| Cover Type | D | A | A |
| Hc (Shore D) | 60 | 29 | 29 |
| Tc (mm) | 0.5 | 0.5 | 0.5 |
| Hm2 - Hm1 | 9 | 0 | 0 |
| Hm2 - Hc | -4 | 36 | 18 |
| T1 + T2 (mm) | 1.6 | 1.6 | 1.6 |

| Ball | | | |
|---|---|---|---|
| Db (mm) | 2.6 | 2.6 | 2.6 |
| (W#1) spin (rpm) | 2750 | 2900 | 3350 |
| (W#1) flight(m) | 249 | 246 | 233 |
| (SW) spin (rpm) | 5700 | 6400 | 6950 |
| Durability | 103 | 85 | 128 |

As shown in Tables II-6 to II-11, the golf balls according to Examples are excellent in various performance characteristics. From the results of evaluation, advantages of the present invention are clear.

## Claims

1. A golf ball comprising a spherical core (4), an inner mid layer (6) positioned outside the core (4), an outer mid layer (8) positioned outside the inner mid layer (6), and a cover (12) positioned outside the outer mid layer (8), wherein
the core (4) has a diameter of equal to or greater than 36.0 mm,
when distances (%) from a central point of the core (4) to nine points and JIS-C hardnesses at the nine points, which nine points are obtained by dividing a region from the central point of the core (4) to a surface of the core (4) at intervals of 12.5% of a radius of the core (4), are plotted in a graph, R² of a linear approximation curve obtained by a least-square method is equal to or greater than 0.95,
**characterized in that** either
i) a Shore D hardness Hm1 of the inner mid layer (6) is greater than a Shore D hardness Hm2 of the outer mid layer (8), a Shore D hardness Hc of the cover (12) is less than the hardness Hm1, and a thickness T2 of the outer mid layer (8) is equal to or greater than 0.5 mm but equal to or less than 1.6 mm, or ii) a Shore D hardness Hm2 of the outer mid layer (108) is greater than a Shore D hardness Hm1 of the inner mid layer (106), a Shore D hardness Hc of the cover (112) is less than the hardness Hm2, and the hardness Hm1 is less than 50.

2. The golf ball according to claim 1, wherein for alternative i) a difference (Hm1-Hm2) between the hardness Hm1 and the hardness Hm2 is equal to or greater than 8.

3. The golf ball according to claim 1, wherein for alternative i) a difference (Hm1-Hc) between the hardness Hm1 and the hardness Hc is equal to or greater than 30.

4. The golf ball according to claim 1, wherein for alternative i) the core (4) is obtained by a rubber composition being crosslinked,
the rubber composition includes:
(a) a base rubber;
(b) a co-crosslinking agent;
(c) a crosslinking initiator; and
(d) an acid and/or a salt, wherein the acid and/or salt excludes the co-crosslinking agent, and
the co-crosslinking agent (b) is:
(b1) an α,β-unsaturated carboxylic acid having 3 to 8 carbon atoms; and/or
(b2) a metal salt of an α,β-unsaturated carboxylic acid having 3 to 8 carbon atoms.

5. The golf ball according to claim 1, wherein for alternative ii) a difference (Hm2-Hm1) between the hardness Hm2 and the hardness Hm1 is equal to or greater than 10.

6. The golf ball according to claim 1, wherein for alternative ii) a difference (Hm2-Hc) between the hardness Hm2 and the hardness Hc is equal to or greater than 30.

7. The golf ball according to claim 1, wherein for alternative ii) the core (104) is obtained by a rubber composition being crosslinked,
the rubber composition includes:
(a) a base rubber;
(b) a co-crosslinking agent;
(c) a crosslinking initiator; and
(d) an acid and/or a salt, wherein the acid and/or salt excludes the co-crosslinking agent, and
the co-crosslinking agent (b) is:
(b1) an α,β-unsaturated carboxylic acid having 3 to 8 carbon atoms; and/or
(b2) a metal salt of an α,β-unsaturated carboxylic acid having 3 to 8 carbon atoms.

## Patentansprüche

1. Golfball, umfassend einen kugelförmigen Kern (4), eine innere mittlere Schicht (6), die außerhalb des Kerns (4) angeordnet ist, eine äußere mittlere Schicht (8), die außerhalb der inneren mittleren Schicht (6) angeordnet ist, und eine Abdeckung (12), die außerhalb der äußeren mittleren Schicht (8) angeordnet ist, wobei
der Kern (4) einen Durchmesser von gleich oder größer als 36,0 mm aufweist,
wenn Entfernungen (%) von einem Mittelpunkt des Kerns (4) zu neun Punkten und JIS-C-Härten an den neun Punkten, welche neun Punkte durch Teilen des Bereichs vom Mittelpunkt des Kerns (4) zur Oberfläche des Kerns (4) in Intervallen von 12,5% des Radius des Kerns (4) erhalten werden, in einem Diagramm aufgetragen werden, R² der linearen Näherungskurve, die durch die Methode der kleinsten Quadrate erhalten wird, gleich oder größer als 0,95 ist,
**dadurch gekennzeichnet, dass**
i) eine Shore-D-Härte Hm1 der inneren mittleren Schicht (6) größer als eine Shore-D-Härte Hm2 der äußeren mittleren Schicht (8) ist, eine Shore-D-Härte Hc der Abdeckung (12) kleiner als die Härte Hm1 ist, und eine Dicke T2 der äußeren mittleren Schicht (8) gleich oder größer als 0,5, aber gleich oder kleiner als 1,6 mm ist, oder
ii) eine Shore-D-Härte Hm2 der äußeren mittleren Schicht (108) größer als eine Shore-D-Härte Hm1 der inneren mittleren Schicht (106) ist, eine Shore-D-Härte Hc der Abdeckung (112) kleiner als die Härte Hm2 ist, und die Härte Hm1 kleiner als 50 ist.

2. Golfball nach Anspruch 1, wobei für Alternative i) eine Differenz (Hm1-Hm2) zwischen der Härte Hm1 und der Härte Hm2 gleich oder größer als 8 ist.

3. Golfball nach Anspruch 1, wobei für Alternative i) eine Differenz (Hm1-Hc) zwischen der Härte Hm1 und der Härte Hc gleich oder größer als 30 ist.

4. Golfball nach Anspruch 1, wobei für Alternative i) der Kern (4) durch eine vernetzte Kautschukzusammensetzung erhalten ist,
wobei die Kautschukzusammensetzung umfasst:
(a) einen Basiskautschuk;
(b) ein Co-Vernetzungsmittel;
(c) einen Vernetzungsinitiator; und
(d) eine Säure und/oder ein Salz, wobei die Säure und/oder das Salz das Co-Vernetzungsmittel ausschließt,
wobei das Co-Vernetzungsmittel (b) ist:
(b1) eine α,β-ungesättigte Carbonsäure mit 3 bis 8 Kohlenstoffatomen; und/oder
(b2) ein Metallsalz einer α,β-ungesättigten Carbonsäure mit 3 bis 8 Kohlenstoffatomen.

5. Golfball nach Anspruch 1, wobei für Alternative ii) eine Differenz (Hm2-Hm1) zwischen der Härte Hm2 und der Härte Hm1 gleich oder größer als 10 ist.

6. Golfball nach Anspruch 1, wobei für Alternative ii) eine Differenz (Hm2-Hc) zwischen der Härte Hm2 und der Härte Hc gleich oder größer als 30 ist.

7. Golfball nach Anspruch 1, wobei für Alternative ii) der Kern (104) durch eine vernetzte Kautschukzusammensetzung erhalten ist,
wobei die Kautschukzusammensetzung umfasst:
(a) einen Basiskautschuk;
(b) ein Co-Vernetzungsmittel;
(c) einen Vernetzungsinitiator; und
(d) eine Säure und/oder ein Salz, wobei die Säure und/oder das Salz das Co-Vernetzungsmittel ausschließt,
wobei das Co-Vernetzungsmittel (b) ist:
(b1) eine α,β-ungesättigte Carbonsäure mit 3 bis 8 Kohlenstoffatomen; und/oder
(b2) ein Metallsalz einer α,β-ungesättigten Carbonsäure mit 3 bis 8 Kohlenstoffatomen.

## Revendications

1. Balle de golf comprenant un cœur sphérique (4), une couche moyenne interne (6) positionnée à l'extérieur du cœur (4), une couche moyenne externe (8) positionnée à l'extérieur de la couche moyenne interne (6), et un couvercle (12) positionné à l'extérieur de la couche moyenne externe (8), le cœur (4) ayant un diamètre supérieur ou égal à 36,0 mm,
lorsque les distances (%) d'un point central du cœur (4) à neuf points et les duretés JIS-C aux neuf points, lesquels neuf points sont obtenus en divisant une région du point central du cœur (4) à une surface du cœur (4) à des intervalles de 12,5 % d'un rayon du cœur (4), sont portés sur un graphe, R² d'une courbe d'approximation linéaire obtenue par une méthode des moindres carrés est supérieur ou égal à 0,95,
**caractérisé en ce que**
i) une dureté D Shore Hm1 de la couche moyenne interne (6) est supérieure à une dureté D Shore Hm2 de la couche moyenne externe (8), une dureté D Shore Hc du couvercle (12) est inférieure à la dureté Hm1, et une épaisseur T2 de la couche moyenne externe (8) est supérieure ou égale à 0,5 mm mais inférieure ou égale à 1,6 mm, ou
ii) une dureté D Shore Hm2 de la couche moyenne externe (108) est supérieure à une dureté D Shore Hm1 de la couche moyenne interne (106), une dureté D Shore Hc du couvercle (112) est inférieure à la dureté Hm2, et la dureté Hm1 est inférieure à 50.

2. Balle de golf selon la revendication 1, dans laquelle pour l'alternative i) une différence (Hm1 - Hm2) entre la dureté Hm1 et la dureté Hm2 est supérieure ou égale à 8.

3. Balle de golf selon la revendication 1, dans laquelle pour l'alternative i) une différence (Hm1 - Hc) entre la dureté Hm1 et la dureté Hc est supérieure ou égale à 30.

4. Balle de golf selon la revendication 1, dans laquelle pour l'alternative i) le cœur (4) est obtenu par une composition de caoutchouc qui est réticulée, la composition de caoutchouc comprend :
(a) un caoutchouc de base ;
(b) un agent de co-réticulation ;
(c) un initiateur de réticulation ; et
(d) un acide et/ou un sel, l'acide et/ou le sel excluant l'agent de co-réticulation, et
l'agent de co-réticulation (b) est :
(b1) un acide carboxylique α,β-insaturé ayant 3 à 8 atomes de carbone ; et/ou
(b2) un sel métallique d'un acide carboxylique α,β-insaturé ayant 3 à 8 atomes de carbone.

5. Balle de golf selon la revendication 1, dans laquelle pour l'alternative ii) une différence (Hm2 - Hm1) entre la dureté Hm2 et la dureté Hm1 est supérieure ou égale à 10.

6. Balle de golf selon la revendication 1, dans laquelle pour l'alternative ii) une différence (Hm2 - Hc) entre la dureté Hm2 et la dureté Hc est supérieure ou égale à 30.

7. Balle de golf selon la revendication 1, dans laquelle pour l'alternative ii) le cœur (104) est obtenu par une composition de caoutchouc qui est réticulée, la composition de caoutchouc comprend :
(a) un caoutchouc de base ;
(b) un agent de co-réticulation ;
(c) un initiateur de réticulation ; et
(d) un acide et/ou un sel, l'acide et/ou le sel excluant l'agent de co-réticulation, et
l'agent de co-réticulation (b) est :
(b1) un acide carboxylique α,β-insaturé ayant 3 à 8 atomes de carbone ; et/ou
(b2) un sel métallique d'un acide carboxylique α,β-insaturé ayant 3 à 8 atomes de carbone.
